



US010364478B2

(12) **United States Patent**  
**Yokoi et al.**

(10) **Patent No.:** **US 10,364,478 B2**  
(b4) **Date of Patent:** **Jul. 30, 2019**

(54) **BAINITE-CONTAINING-TYPE HIGH-STRENGTH HOT-ROLLED STEEL SHEET HAVING EXCELLENT ISOTROPIC WORKABILITY AND MANUFACTURING METHOD THEREOF**

(71) **Applicant:** **NIPPON STEEL & SUMITOMO METAL CORPORATION**, Tokyo (JP)

(72) **Inventors:** **Tatsuo Yokoi**, Tokyo (JP); **Hiroshi Shuto**, Tokyo (JP); **Riki Okamoto**, Tokyo (JP); **Nobuhiro Fujita**, Tokyo (JP); **Kazuaki Nakano**, Tokyo (JP); **Takeshi Yamamoto**, Tokyo (JP)

(73) **Assignee:** **NIPPON STEEL CORPORATION**, Tokyo (JP)

(\*) **Notice:** Subject to any disclaimer, the term of this patent is extended or adjusted under 35 U.S.C. 154(b) by 348 days.

(21) **Appl. No.:** **15/411,372**

(22) **Filed:** **Jan. 20, 2017**

(65) **Prior Publication Data**

US 2017/0130294 A1 May 11, 2017

**Related U.S. Application Data**

(62) Division of application No. 13/985,001, filed as application No. PCT/JP2012/058337 on Mar. 29, 2012, now Pat. No. 9,587,287.

(30) **Foreign Application Priority Data**

Mar. 31, 2011 (JP) ..... 2011-079658

(51) **Int. Cl.**

**C21D 9/46** (2006.01)  
**C21D 8/02** (2006.01)  
**C22C 38/06** (2006.01)  
**C22C 38/58** (2006.01)  
**C22C 38/00** (2006.01)  
**C22C 38/02** (2006.01)  
**C22C 38/04** (2006.01)  
**C22C 38/08** (2006.01)  
**C22C 38/12** (2006.01)  
**C22C 38/14** (2006.01)  
**C22C 38/16** (2006.01)  
**C22C 38/28** (2006.01)  
**C22C 38/38** (2006.01)  
**C22C 38/18** (2006.01)  
**C21D 6/00** (2006.01)

(52) **U.S. Cl.**

CPC ..... **C21D 9/46** (2013.01); **C21D 6/002** (2013.01); **C21D 6/005** (2013.01); **C21D 6/008** (2013.01); **C21D 8/02** (2013.01); **C21D 8/0205** (2013.01); **C21D 8/0226** (2013.01); **C21D 8/0263** (2013.01); **C22C 38/001** (2013.01); **C22C 38/002** (2013.01); **C22C 38/005** (2013.01); **C22C 38/02** (2013.01); **C22C 38/04** (2013.01); **C22C 38/06** (2013.01);

**C22C 38/08** (2013.01); **C22C 38/12** (2013.01); **C22C 38/14** (2013.01); **C22C 38/16** (2013.01); **C22C 38/18** (2013.01); **C22C 38/28** (2013.01); **C22C 38/38** (2013.01); **C22C 38/58** (2013.01); **C21D 2201/05** (2013.01); **C21D 2211/002** (2013.01); **C21D 2211/005** (2013.01)

(58) **Field of Classification Search**

None  
See application file for complete search history.

(56) **References Cited**

**U.S. PATENT DOCUMENTS**

|                 |         |                |
|-----------------|---------|----------------|
| 2003/0196735 A1 | 10/2003 | Sugiura et al. |
| 2004/0244877 A1 | 12/2004 | Yokoi et al.   |
| 2007/0089814 A1 | 4/2007  | Sugiura et al. |
| 2009/0032148 A1 | 2/2009  | Kozuma et al.  |

**FOREIGN PATENT DOCUMENTS**

|    |            |         |
|----|------------|---------|
| CN | 1462317 A  | 12/2003 |
| CN | 1599802 A  | 3/2005  |
| CN | 1809646 A  | 7/2006  |
| EP | 1327695 A1 | 7/2003  |

(Continued)

**OTHER PUBLICATIONS**

Mexican Office Action, dated Jun. 22, 2017, for corresponding Mexican Application No. MX/a/2013/009507, with a partial English translation.

International Search Report issued in PCT/JP2012/058337, dated Jun. 26, 2012.

Taiwanese Office Action dated Feb. 24, 2014, issued in corresponding Taiwanese Patent Application No. 101111104.

Written Opinion of the International Searching Authority issued in PCT/JP2012/058337, dated Jun. 26, 2012.

Chinese Office Action and Search Report, dated Nov. 25, 2014, for Chinese Application No. 201280014599.3.

(Continued)

*Primary Examiner* — Jenny R Wu

(74) **Attorney, Agent, or Firm:** Birch, Stewart, Kolasch & Birch, LLP

(57) **ABSTRACT**

The present invention provides a bainite-containing-type high-strength hot-rolled steel sheet. The steel sheet, containing C: greater than 0.07 to 0.2%, Si: 0.001 to 2.5%, Mn: 0.01 to 4%, P: 0.15% or less, S: 0.03% or less, N: 0.01% or less, Al: 0.001 to 2% and a balance being composed of Fe and impurities, has an average value of pole densities of the {100}<011> to {223}<110> orientation group at a sheet thickness center portion being a range of  $\frac{5}{8}$  to  $\frac{3}{8}$  in sheet thickness from the surface of the steel sheet is 4.0 or less, and a pole density of the {332}<113> crystal orientation is 4.8 or less, an average crystal grain diameter is 10  $\mu\text{m}$  or less and vTrs is  $-20^\circ\text{C}$ . or lower, and a microstructure is composed of 35% or less in a structural fraction of proeutectoid ferrite and a balance of a low-temperature transformation generating phase.

(56)

**References Cited**

|    |             |    |         |
|----|-------------|----|---------|
| JP | 2009-263718 | A  | 11/2009 |
| TW | 2005-17507  |    | 6/1993  |
| WO | WO 99/05335 | A1 | 2/1999  |

**FOREIGN PATENT DOCUMENTS**

|    |             |   |         |
|----|-------------|---|---------|
| JP | 6-293910    | A | 10/1994 |
| JP | 10-183255   | A | 7/1998  |
| JP | 2002-115025 | A | 4/2002  |
| JP | 2002-322540 | A | 11/2002 |
| JP | 2002-322541 | A | 11/2002 |
| JP | 2002-363695 | A | 12/2002 |
| JP | 2005-15854  | A | 1/2005  |
| JP | 2006-124789 | A | 5/2006  |
| JP | 2008-69425  | A | 3/2008  |
| JP | 2009-19265  | A | 1/2009  |
| JP | 2009-30159  | A | 2/2009  |

**OTHER PUBLICATIONS**

Non-Final Office Action dated Jun. 15, 2016, issued in U.S. Appl. No. 13/985,001.  
Notice of Allowance dated Oct. 28, 2016, issued in U.S. Appl. No. 13/985,001.  
Brazilian Office Action and Search Report, dated Oct. 30, 2018, for corresponding Brazilian Application No. BR112013024166-7, with an English translation.  
Indian Office Action, dated Dec. 4, 2018, for corresponding Indian Application No. 7672/DELNP/2013, with an English translation.

FIG.1



FIG.2



FIG.3



FIG.4



**BAINITE-CONTAINING-TYPE  
HIGH-STRENGTH HOT-ROLLED STEEL  
SHEET HAVING EXCELLENT ISOTROPIC  
WORKABILITY AND MANUFACTURING  
METHOD THEREOF**

This application is a Divisional of U.S. patent application Ser. No. 13/985,001, filed on Aug. 12, 2013, which is the U.S. National Phase of PCT/JP2012/058337, filed Mar. 29, 2012, which claims priority under 35 U.S.C. § 119(a) to Patent Application No. JP 2011-079658, filed in Japan on Mar. 31, 2011, all of which are hereby expressly incorporated by reference into the present application.

**TECHNICAL FIELD**

The present invention relates to a bainite-containing-type high-strength hot-rolled steel sheet having excellent isotropic workability and a manufacturing method thereof.

**BACKGROUND ART**

In recent years, for weight reduction in various members with the aim of improving fuel efficiency of an automobile, a reduction in thickness by achieving high strength of a steel sheet of iron alloy or the like and application of light metal such as Al alloy have been promoted. However, as compared to heavy metal such as steel, the light metal such as Al alloy has the advantage of specific strength being high, but has the disadvantage of being expensive significantly. Therefore, the application of light metal such as Al alloy has been limited to special use. Thus, in order to promote the weight reduction in various members more inexpensively and widely, the reduction in thickness by achieving high strength of a steel sheet has been needed.

The achievement of high strength of a steel sheet causes deterioration of material properties such as formability (workability) in general. Therefore, how the achievement of high strength is attained without deteriorating the material properties is important in developing a high-strength steel sheet. Particularly, a steel sheet used as an automobile member such as an inner sheet member, a structure member, or an underbody member is required to have bendability, stretch flange workability, burring workability, ductility, fatigue durability, impact resistance, corrosion resistance, and so on according to its use. It is important how these material properties and high strength property should be exhibited in a high-dimensional and well-balanced manner.

Particularly, among automobile parts, a part obtained by working a sheet material as a raw material and exhibiting a function as a rotor, such as a drum or a carrier constituting an automatic transmission, for example, is an important part serving as a mediator of transmitting engine output to an axle shaft. Such a part exhibiting a function as a rotor is required to have circularity as a shape and sheet thickness homogeneity in a circumferential direction in order to decrease friction and the like. Further, for forming such a part, forming methods such as burring, drawing, ironing, and bulging are used, and a great emphasis is placed also on ultimate ductility typified by local elongation.

Further, with regard to a steel sheet used for such a member, it is necessary to improve a property that the steel sheet is formed and then is attached to an automobile as a part and then the member is not easily broken even when being subjected to impact caused by collision or the like. Further, in order to secure the impact resistance in a cold district, it is also necessary to improve low-temperature

toughness. This low-temperature toughness is defined by vTrs (a Charpy fracture appearance transition temperature), or the like. For this reason, it is also necessary to consider the impact resistance itself of the above-described steel member.

That is, a thin steel sheet for a part required to have sheet thickness uniformity such as the above-described part is required to have, in addition to excellent workability, plastic isotropy and low-temperature toughness as very important properties.

In order to achieve the high strength property and the various material properties such as formability in particular as above, in Patent Document 1, for example, there has been disclosed a manufacturing method of a steel sheet in which

15 a steel structure is made of 90% or more of ferrite and a balance of bainite, to thereby achieve high strength, ductility, and bore expandability. However, with regard to a steel sheet manufactured by applying the technique disclosed in Patent Document 1, the plastic isotropy is not mentioned at

20 all. On the condition that the steel sheet manufactured in Patent Document 1 is applied to a part required to have circularity and sheet thickness homogeneity in a circumferential direction, a decrease in output due to false vibration and/or friction loss caused by an eccentricity of the part is concerned.

Further, in Patent Documents 2 and 3, there has been disclosed a technique of a high-tensile hot-rolled steel sheet to which high strength and excellent stretch flange formability are provided by adding Mo and making precipitates fine.

30 However, a steel sheet to which the techniques disclosed in Patent Documents 2 and 3 are applied is required to have 0.07% or more of Mo being an expensive alloy element added thereto, and thus has a problem that its manufacturing cost is high. Further, in the techniques disclosed in Patent Documents 2 and 3 as well, the plastic isotropy is not mentioned at all. On the condition that the techniques in Patent Documents 2 and 3 are also applied to a part required to have circularity and sheet thickness homogeneity in a circumferential direction, a decrease in

35 output due to false vibration and/or friction loss caused by an eccentricity of the part is concerned.

On the other hand, with regard to the plastic isotropy of the steel sheet, namely a decrease in plastic anisotropy, in Patent Document 4, for example, there has been disclosed a

40 technique in which endless rolling and lubricated rolling are combined, and thereby a texture of austenite in a shear layer of a surface layer is regulated and in-plane anisotropy of an r value (Lankford value) is decreased. However, in order to perform the lubricated rolling with a small friction coefficient over an entire length of a coil, the endless rolling is needed for preventing biting failure caused by slip between a roll bite and a rolled sheet material during rolling. However, in order to apply this technique, investment in facilities such as a rough bar joining apparatus, a high-speed crop shear, and so on is needed and thus a burden is large.

Further, in Patent Document 5, for example, there has been disclosed a technique in which Zr, Ti, and Mo are compositely added and finish rolling is finished at a high temperature of 950° C. or higher, and thereby strength of

60 780 MPa class or more is obtained, anisotropy of an r value is small, and stretch flange formability and deep drawability are achieved. However, 0.1% or more of Mo being an expensive alloy element is needed to be added, and thus there is a problem that its manufacturing cost is high.

65 Further, a study of improving the low-temperature toughness of a steel sheet has been advanced up to now, but a bainite-containing-type high-strength hot-rolled steel sheet

having excellent isotropic workability that has high strength, exhibits plastic isotropy, improves hole expandability, and further achieves also low-temperature toughness has not been disclosed in Patent Documents 1 to 5.

## PRIOR ART DOCUMENT

## Patent Document

Patent Document 1: Japanese Laid-open Patent Publication No. H6-293910

Patent Document 2: Japanese Laid-open Patent Publication No. 2002-322540

Patent Document 3: Japanese Laid-open Patent Publication No. 2002-322541

Patent Document 4: Japanese Laid-open Patent Publication No. H10-183255

Patent Document 5: Japanese Laid-open Patent Publication No. 2006-124789

## DISCLOSURE OF THE INVENTION

## Problems to be Solved by the Invention

The present invention has been invented in consideration of the above-described problems, and has an object to provide a bainite-containing-type high-strength hot-rolled steel sheet having excellent isotropic workability that has high strength, is applicable to a member required to have workability, hole expandability, bendability, strict sheet thickness uniformity and circularity after working, and low-temperature toughness, and has a steel sheet grade of 540 MPa class or more, and a manufacturing method capable of manufacturing the steel sheet inexpensively and stably.

## Means for Solving the Problems

In order to solve the problems as described above, the present inventors propose a bainite-containing-type high-strength hot-rolled steel sheet having excellent isotropic workability and a manufacturing method described below.

[1]

A bainite-containing-type high-strength hot-rolled steel sheet having excellent isotropic workability, contains:

in mass %,

C: greater than 0.07 to 0.2%;

Si: 0.001 to 2.5%;

Mn: 0.01 to 4%;

P: 0.15% or less (not including 0%);

S: 0.03% or less (not including 0%);

N: 0.01% or less (not including 0%);

Al: 0.001 to 2%; and

a balance being composed of Fe and inevitable impurities, in which

an average value of pole densities of the  $\{100\}<011>$  to  $\{223\}<110>$  orientation group represented by respective

crystal orientations of  $\{100\}<011>$ ,  $\{116\}<110>$ ,

$\{114\}<110>$ ,  $\{113\}<110>$ ,  $\{112\}<110>$ ,  $\{335\}<110>$ ,

and  $\{223\}<110>$  at a sheet thickness center portion being

a range of  $\frac{1}{8}$  to  $\frac{3}{8}$  in sheet thickness from the surface of

the steel sheet is 4.0 or less, and a pole density of the

$\{332\}<113>$  crystal orientation is 4.8 or less, an average

crystal grain diameter is 10  $\mu\text{m}$  or less and a Charpy

fracture appearance transition temperature  $v_{\text{Trs}}$  is  $-20^\circ\text{C}$ .

or lower, and

a microstructure is composed of 35% or less in a structural fraction of pro-eutectoid ferrite and a balance of a low-temperature transformation generating phase.

[2]

The bainite-containing-type high-strength hot-rolled steel sheet having excellent isotropic workability according to [1], further contains:

one type or two or more types of in mass %,

10 Ti: 0.015 to 0.18%,

Nb: 0.005 to 0.06%,

Cu: 0.02 to 1.2%,

Ni: 0.01 to 0.6%,

Mo: 0.01 to 1%,

15 V: 0.01 to 0.2%, and

Cr: 0.01 to 2%.

[3]

The bainite-containing-type high-strength hot-rolled steel sheet having excellent isotropic workability according to [1], further contains:

one type or two or more types of in mass %,

Mg: 0.0005 to 0.01%,

Ca: 0.0005 to 0.01%, and

25 REM: 0.0005 to 0.1%.

[4]

The bainite-containing-type high-strength hot-rolled steel sheet having excellent isotropic workability according to [1], further contains:

30 in mass %,

B: 0.0002 to 0.002%.

[5]

A manufacturing method of a bainite-containing-type high-strength hot-rolled steel sheet having excellent isotropic workability, includes:

on a steel billet containing:

in mass %,

C: greater than 0.07 to 0.2%;

Si: 0.001 to 2.5%;

40 Mn: 0.01 to 4%;

P: 0.15% or less (not including 0%);

S: 0.03% or less (not including 0%);

N: 0.01% or less (not including 0%);

Al: 0.001 to 2%; and

45 a balance being composed of Fe and inevitable impurities, performing first hot rolling in which rolling at a reduction ratio of 40% or more is performed one time or more in a temperature range of not lower than  $1000^\circ\text{C}$ . nor higher than  $1200^\circ\text{C}$ .;

50 performing second hot rolling in which rolling at 30% or more is performed in one pass at least one time in a temperature region of not lower than  $T_1+30^\circ\text{C}$ . nor higher than  $T_1+200^\circ\text{C}$ . determined by Expression (1) below; and setting the total of reduction ratios in the second hot rolling to 50% or more; performing final reduction at a reduction ratio of 30% or more in the second hot rolling and then starting primary cooling in a manner that a waiting time period  $t$  second satisfies Expression (2) below;

55 setting an average cooling rate in the primary cooling to  $50^\circ\text{C./second}$  or more and performing the primary cooling in a manner that a temperature change is in a range of not lower than  $40^\circ\text{C}$ . nor higher than  $140^\circ\text{C}$ .;

60 within three seconds after completion of the primary cooling, performing secondary cooling in which cooling is performed at an average cooling rate of  $15^\circ\text{C./second}$  or more; and

## 5

after completion of the secondary cooling, performing air cooling for 1 to 20 seconds in a temperature region of lower than an Ar3 transformation point temperature and an Ar1 transformation point temperature or higher and next performing coiling at 450° C. or higher and lower than 550° C.

$$T1(\text{° C.}) = 850 + 10 \times (C + N) \times Mn + 350 \times Nb + 250 \times Ti + 40 \times B + 10 \times Cr + 100 \times Mo + 100 \times V \quad (1)$$

Here, C, N, Mn, Nb, Ti, B, Cr, Mo, and V each represent the content of the element (mass %).

$$t = 2.5 \times t1 \quad (2)$$

Here,  $t_1$  is obtained by Expression (3) below.

$$t1 = 0.001 \times ((Tf - T1) \times P1 / 100)^2 - 0.109 \times ((Tf - T1) \times P1 / 100) + 3.1 \quad (3)$$

Here, in Expression (3) above,  $T_f$  represents the temperature of the steel billet obtained after the final reduction at a reduction ratio of 30% or more, and  $P_1$  represents the reduction ratio of the final reduction at 30% or more.

[6]

The manufacturing method of the bainite-containing-type high-strength hot-rolled steel sheet having excellent isotropic workability according to [5], in which the total of reduction ratios in a temperature range of lower than  $T1 + 30^\circ \text{C.}$  is 30% or less.

[7]

The manufacturing method of the bainite-containing-type high-strength hot-rolled steel sheet having excellent isotropic workability according to [5], in which heat generation by working between respective passes in the temperature region of not lower than  $T1 + 30^\circ \text{C.}$  nor higher than  $T1 + 200^\circ \text{C.}$  in the second hot rolling is  $18^\circ \text{C.}$  or lower.

[8]

The manufacturing method of the bainite-containing-type high-strength hot-rolled steel sheet having excellent isotropic workability according to [5], in which the waiting time period  $t$  second further satisfies Expression (4) below.

$$t < t1 \quad (4)$$

[9]

The manufacturing method of the bainite-containing-type high-strength hot-rolled steel sheet having excellent isotropic workability according to [5], in which the waiting time period  $t$  second further satisfies Expression (5) below.

$$t1 \leq t \leq t1 \times 2.5 \quad (5)$$

[10]

The manufacturing method of the bainite-containing-type high-strength hot-rolled steel sheet having excellent isotropic workability according to [5], in which the primary cooling is started between rolling stands.

### Effect of the Invention

According to the present invention, there is provided a steel sheet applicable to a member required to have workability, hole expandability, bendability, strict sheet thickness uniformity and circularity after working, and low-temperature toughness (an inner sheet member, a structure member, an underbody member, an automobile member such as a transmission, and members for shipbuilding, construction, bridges, offshore structures, pressure vessels, line pipes, and machine parts, and so on). Further, according to the present

## 6

invention, there is manufactured a high-strength steel sheet having excellent low-temperature toughness and 540 MPa class or more inexpensively and stably.

### BRIEF DESCRIPTION OF THE DRAWINGS

FIG. 1 is a view showing the relationship between an average value of pole densities of the  $\{100\} <011>$  to  $\{223\} <110>$  orientation group and isotropy ( $1/\Delta r$ );

FIG. 2 is a view showing the relationship between a pole density of the  $\{332\} <113>$  crystal orientation and an isotropic index ( $1/\Delta r$ );

FIG. 3 is a view showing the relationship between an average crystal grain diameter ( $\mu\text{m}$ ) and  $v_{Trs}$  ( $^\circ \text{C.}$ ); and

FIG. 4 is an explanatory view of a continuous hot rolling line.

### MODE FOR CARRYING OUT THE INVENTION

As an embodiment implementing the present invention, there will be explained a bainite-containing-type high-strength hot-rolled steel sheet having excellent isotropic workability, (which will be simply called a "hot-rolled steel sheet" hereinafter), in detail. Incidentally, mass % related to a chemical composition is simply described as %.

The present inventors earnestly studied the bainite-containing-type high-strength hot-rolled steel sheet suitable for application to a member required to have workability, hole expandability, bendability, strict sheet thickness uniformity and circularity after working, and low-temperature toughness, in terms of workability and further achievement of isotropy and low-temperature toughness. As a result, the following new knowledge was obtained.

First, for obtaining the isotropy (decreasing anisotropy), formation of a transformation texture from non-recrystallized austenite, being the cause of anisotropy, is avoided. In order to achieve it, it is necessary to promote recrystallization of austenite after finish rolling. As its means, an optimum rolling pass schedule in finish rolling and achievement of high temperature of a rolling temperature are effective.

Next, for improving the low-temperature toughness, making grains fine in each fracture of a brittle fracture, namely grain refining in each microstructure is effective. For this, it is effective to increase nucleation sites for  $\alpha$  at the time of transformation of  $\gamma$  to  $\alpha$ , and it becomes necessary to increase crystal grain boundaries of austenite that can be the nucleation sites and dislocation density.

As its means, it becomes necessary to perform rolling at a  $\gamma$  to  $\alpha$  transformation point temperature or higher and at as low a temperature as possible, namely to make austenite remain non-recrystallized and in a state of a non-recrystallization fraction being high, cause the  $\gamma$  to  $\alpha$  transformation.

This is because austenite grains after recrystallization grow quickly at a recrystallization temperature, become coarse for an extremely short time, and become coarse even in a phase after the  $\gamma$  to  $\alpha$  transformation to thereby cause significant toughness deterioration.

The present inventors invented an entirely new hot rolling method capable of, on a higher level, balancing the isotropy and the low-temperature toughness, which were considered difficult to be achieved because they resulted in conditions opposite to each other by a normal hot rolling means.

First, as for the isotropy, the present inventors obtained the following knowledge with regard to the relationship between isotropy and texture.

In order to obtain the sheet thickness uniformity and circularity that satisfy a part property in a state where the steel sheet remains worked without being subjected to trimming and cutting processes, at least an isotropic index ( $=1/|\Delta r|$ ) is needed to be 3.5 or more.

Here, the isotropic index is obtained in a manner that the steel sheet is worked into a No. 5 test piece described in JIS Z 2201 and the test piece is subjected to a test by the method described in JIS Z 2241.  $1/|\Delta r|$  being the isotropic index is defined as  $\Delta r = (rL - 2x r45 + rC)/2$ , where plastic strain ratios ( $r$  values: Lankford values) in a rolling direction, in a  $45^\circ$  direction with respect to the rolling direction, and in a  $90^\circ$  direction with respect to the rolling direction (sheet width direction) are defined as  $rL$ ,  $r45$ , and  $rC$  respectively.

(Crystal Orientation)

As shown in FIG. 1, the isotropic index ( $=1/|\Delta r|$ ) satisfies 3.5 or more as long as an average value of pole densities of the  $\{100\}<011>$  to  $\{223\}<110>$  orientation group represented by respective crystal orientations of  $\{100\}<011>$ ,  $\{116\}<110>$ ,  $\{114\}<110>$ ,  $\{113\}<110>$ ,  $\{112\}<110>$ ,  $\{335\}<110>$ , and  $\{223\}<110>$  at a sheet thickness center portion being a range of  $\frac{1}{8}$  to  $\frac{3}{8}$  in sheet thickness from the surface of the steel sheet is 4.0 or less. As long as the isotropic index is 6.0 or more desirably, the sheet thickness uniformity and circularity that sufficiently satisfy the part property in a state where the steel sheet remains worked can be obtained even though variations in a coil are considered. Therefore, the average value of the pole densities of the  $\{100\}<011>$  to  $\{223\}<110>$  orientation group is desirably 2.0 or less.

The pole density is synonymous with an X-ray random intensity ratio. The pole density (X-ray random intensity ratio) is a numerical value obtained by measuring X-ray intensities of a standard sample not having concentration in a specific orientation and a test sample under the same conditions by X-ray diffractometry or the like and dividing the obtained X-ray intensity of the test sample by the X-ray intensity of the standard sample. This pole density can be measured by any one of X-ray diffractometry, an EBSP (Electron Back Scattering Pattern) method, and an ECP (Electron Channeling Pattern) method.

As for the pole density of the  $\{100\}<011>$  to  $\{223\}<110>$  orientation group, for example, pole densities of respective orientations of  $\{100\}<011>$ ,  $\{116\}<110>$ ,  $\{114\}<110>$ ,  $\{112\}<110>$ , and  $\{223\}<110>$  are obtained from a three-dimensional texture (ODF) calculated by a series expansion method using a plurality (preferably three or more) of pole figures out of pole figures of  $\{110\}$ ,  $\{100\}$ ,  $\{211\}$ , and  $\{310\}$  measured by the method, and these pole densities are arithmetically averaged, and thereby the pole density of the above-described orientation group is obtained. Incidentally, when it is impossible to obtain the intensities of all the above-described orientations, the arithmetic average of the pole densities of the respective orientations of  $\{100\}<011>$ ,  $\{116\}<110>$ ,  $\{114\}<110>$ ,  $\{112\}<110>$ , and  $\{223\}<110>$  may also be used as a substitute.

For example, for the pole density of each of the above-described crystal orientations, each of intensities of  $(001)[1-10]$ ,  $(116)[1-10]$ ,  $(114)[1-10]$ ,  $(113)[1-10]$ ,  $(112)[1-10]$ ,  $(335)[1-10]$ , and  $(223)[1-10]$  at a  $\phi=45^\circ$  cross-section in the three-dimensional texture may be used as it is.

Similarly, as shown in FIG. 2, as long as the pole density of the  $\{332\}<113>$  crystal orientation at the sheet thickness center portion being the range of  $\frac{1}{8}$  to  $\frac{3}{8}$  in sheet thickness from the surface of the steel sheet is 4.8 or less, the isotropic index satisfies 3.5 or more. As long as the isotropic index is 6.0 or more desirably, the sheet thickness uniformity and

circularity that sufficiently satisfy the part property in a state where the steel sheet remains worked can be obtained even though variations in a coil are considered. Therefore, the pole density of the  $\{332\}<113>$  crystal orientation is desirably 3.0 or less.

With regard to the sample to be subjected to the X-ray diffractometry, EBSP method, or ECP method, the steel sheet is reduced in thickness to a predetermined sheet thickness from the surface by mechanical polishing or the like. Next, strain is removed by chemical polishing, electrolytic polishing, or the like, and the sample is manufactured in such a manner that in the range of  $\frac{1}{8}$  to  $\frac{3}{8}$  in sheet thickness, an appropriate plane becomes a measuring plane. For example, on a steel piece in a size of 30 mm<sup>2</sup> cut out from the position of  $\frac{1}{4}W$  or  $\frac{3}{4}W$  of the sheet width  $W$ , grinding with fine finishing (centerline average roughness  $R_a$ : 0.4 a to 1.6 a) is performed. Next, by chemical polishing or electrolytic polishing, strain is removed, and the sample to be subjected to the X-ray diffractometry is manufactured. With regard to the sheet width direction, the steel piece is desirably taken from, of the steel sheet, the position of  $\frac{1}{4}$  or  $\frac{3}{4}$  from an end portion.

As a matter of course, the pole density satisfies the above-described pole density limited range not only at the sheet thickness center portion being the range of  $\frac{1}{8}$  to  $\frac{3}{8}$  in sheet thickness from the surface of the steel sheet, but also at as many thickness positions as possible, and thereby local ductile performance (local elongation) is further improved. However, the range of  $\frac{1}{8}$  to  $\frac{3}{8}$  from the surface of the steel sheet is measured, to thereby make it possible to represent the material property of the entire steel sheet generally. Thus,  $\frac{1}{8}$  to  $\frac{3}{8}$  of the sheet thickness is defined as the measuring range.

Incidentally, the crystal orientation represented by  $\{hkl\}<uvw>$  means that the normal direction of the steel sheet plane is parallel to  $\{hkl\}$  and the rolling direction is parallel to  $\langle uvw \rangle$ . With regard to the crystal orientation, normally, the orientation vertical to the sheet plane is represented by  $[hkl]$  or  $\{hkl\}$  and the orientation parallel to the rolling direction is represented by  $(uvw)$  or  $\langle uvw \rangle$ .  $\{hkl\}$ ,  $\langle uvw \rangle$ , and so on are generic terms for equivalent planes, and  $[hkl]$ ,  $(uvw)$  each indicate an individual crystal plane. That is, in the present invention, a body-centered cubic structure is targeted, and thus, for example, the  $(111)$ ,  $(-111)$ ,  $(1-11)$ ,  $(11-1)$ ,  $(-1-11)$ ,  $(-11-1)$ ,  $(1-1-1)$ , and  $(-1-1-1)$  planes are equivalent to make it impossible to make them different. In such a case, these orientations are generically referred to as  $\{111\}$ . In an ODF representation,  $[hkl](uvw)$  is also used for representing orientations of other low symmetric crystal structures, and thus it is general to represent each orientation as  $[hkl](uvw)$ , but in the present invention,  $[hkl](uvw)$  and  $\{hkl\}<uvw>$  are synonymous with each other. The measurement of crystal orientation by an X ray is performed according to the method described in, for example, Cullity, Elements of X-ray Diffraction, new edition (published in 1986, translated by MATSUMURA, Gentaro, published by AGNE Inc.) on pages 274 to 296.

(Average Crystal Grain Diameter)

Next, the present inventors examined the low-temperature toughness.

FIG. 3 shows the relationship between an average crystal grain diameter and  $v_{Trs}$  (a Charpy fracture appearance transition temperature). As the average crystal grain diameter is smaller,  $v_{Trs}$  becomes low in temperature, and the toughness at low temperature is improved. As long as the average crystal grain diameter is 10  $\mu\text{m}$  or less,  $v_{Trs}$

becomes  $-20^{\circ}\text{C}$ . or lower as a target, and thus the present invention is durable enough to be used in a cold district.

Incidentally, the low-temperature toughness was evaluated by vTrs (the Charpy fracture appearance transition temperature) obtained by a V-notch Charpy impact test. In the V-notch Charpy impact test, a test piece was made based on JISZ2202 and the test was performed according to the contents defined in JISZ2242, and vTrs was measured.

Further, the low-temperature toughness is greatly affected by the average crystal grain diameter of the structure, and thus the measurement of the average crystal grain diameter in the sheet thickness center portion was also performed. A microsample was cut out to have a crystal grain diameter and microstructure thereof measured by using EBSP-OIM<sup>TM</sup> (Electron Back Scatter Diffraction Pattern-Orientation Image Microscopy). The microsample was polished by using a colloidal silica abrasive for 30 to 60 minutes to be made and was subjected to an EBSP measurement under measurement conditions of 400 magnifications,  $160\text{ }\mu\text{m}\times 256$   $\mu\text{m}$  area, and a measurement step of  $0.5\text{ }\mu\text{m}$ .

The EBSP-OIM<sup>TM</sup> method is constituted by a device and software that a highly inclined sample in a scanning electron microscope (SEM) is irradiated with electron beams, a Kikuchi pattern formed by backscattering is photographed by a high-sensitive camera and is image processed by a computer, and thereby a crystal orientation at an irradiation point is measured for a short time period.

In the EBSP method, it is possible to quantitatively analyze a microstructure and a crystal orientation of a bulk sample surface. An analysis area of the EBSP method is an area capable of being observed by the SEM. It is possible to analyze the area with a minimum resolution of  $20\text{ nm}$  by the EBSP method, depending on the resolution of the SEM. The analysis is performed by mapping an area to be analyzed to tens of thousands of equally-spaced grid points. It is possible to see crystal orientation distributions and sizes of crystal grains within the sample in a polycrystalline material.

In the present invention, from an image mapped in a manner that an orientation difference between crystal grains is defined as  $15^{\circ}$  being a threshold value of a large angle tilt grain boundary recognized as a crystal grain boundary generally, the crystal grains were visualized and the average crystal grain diameter was obtained. Here, the "average crystal grain diameter" is a value obtained by the EBSP-OIM<sup>TM</sup>.

As described above, the present inventors revealed respective requirements necessary for the steel sheet for obtaining the isotropy and the low-temperature toughness.

The average crystal grain diameter directly related to the low-temperature toughness becomes small as a finish rolling finishing temperature is lower, and thus the low-temperature toughness is improved. However, the average value of the pole densities of the  $\{100\}<011>$  to  $\{223\}<110>$  orientation group at the sheet thickness center portion corresponding to  $\frac{1}{8}$  to  $\frac{3}{8}$  from the surface of the steel sheet and the pole density of the  $\{332\}<113>$  crystal orientation, which are one of control factors of the isotropy, are inversely correlated to the average crystal grain diameter. That is, it is the relation in which when the average crystal grain diameter is decreased in order to improve the low-temperature toughness, the average value of the pole densities of the  $\{100\}<011>$  to  $\{223\}<110>$  orientation group and the pole density of the  $\{332\}<113>$  crystal orientation are increased and thus the isotropy deteriorates. The technique achieving the isotropy and the low-temperature toughness has not been disclosed so far at all.

The present inventors earnestly examined the bainite-containing-type high-strength hot-rolled steel sheet suitable for application to a member required to have workability, hole expandability, bendability, strict sheet thickness uniformity and circularity after working, and low-temperature toughness and allowing the isotropy and the low-temperature toughness to be achieved and a manufacturing method thereof. As a result, the present inventors thought of a hot-rolled steel sheet made of the following conditions and a manufacturing method thereof

(Chemical Composition)

First, there will be explained reasons for limiting a chemical composition of the bainite-containing-type high-strength hot-rolled steel sheet of the present invention, which will be sometimes called a "present invention hot-rolled steel sheet" hereinafter.

C: greater than 0.07 to 0.2%

C is an element contributing to increasing the strength of the steel, but is also an element generating iron-based carbide such as cementite ( $\text{Fe}_3\text{C}$ ) to be the starting point of cracking at the time of hole expansion. When C is 0.07% or less, it is not possible to obtain a strength improving effect by a low-temperature transformation generating phase. On the other hand, when C exceeds 0.2%, center segregation becomes noticeable and iron-based carbide such as cementite ( $\text{Fe}_3\text{C}$ ) to be the starting point of cracking in a secondary shear surface at the time of punching is increased, resulting in that a punching property deteriorates. Therefore, C is set to greater than 0.07 to 0.2%. When the balance between strength and ductility is considered, C is desirably 0.15% or less.

Si: 0.001 to 2.5%

Si is an element contributing to increasing the strength of the steel and also has a part as a deoxidizing material of molten steel, and thus is added according to need. When Si is 0.001% or more, the above-described effect is exhibited, but when Si exceeds 2.5%, a strength increasing effect is saturated. Therefore, Si is set to 0.001 to 2.5%.

Further, when being greater than 0.1%, Si, with an increase in the content, suppresses precipitation of iron-based carbide such as cementite and contributes to improving the strength and to improving the hole expandability. However, when Si exceeds 1.0%, an effect of suppressing the precipitation of iron-based carbide is saturated. Therefore, Si is preferably greater than 0.1 to 1.0%.

Mn: 0.01 to 4%

Mn is an element contributing to improving the strength by solid-solution strengthening and quenching strengthening and is added according to need. When Mn is less than 0.01%, its addition effect cannot be obtained, and when Mn exceeds 4%, on the other hand, the addition effect is saturated, and thus Mn is set to 0.01 to 4%.

In order to suppress occurrence of hot cracking by S, when elements other than Mn are not added sufficiently, the Mn amount allowing the Mn amount (mass %) ( $[\text{Mn}]$ ) and the S amount (mass %) ( $[\text{S}]$ ) to satisfy  $[\text{Mn}]/[\text{S}] \geq 20$  is desirably added. Further, Mn is an element that, with an increase in the content, expands an austenite region temperature to a low temperature side, improves the hardenability, and facilitates formation of a continuous cooling transformation structure having excellent burring. When Mn is less than 1%, this effect is not easily exhibited, and thus Mn is desirably 1% or more.

P: 0.15% or less

P is an impurity contained in molten iron, and is an element that is segregated at grain boundaries and decreases the toughness. For this reason, it is desirable as P is smaller,

## 11

and when exceeding 0.15%, P adversely affects the workability and weldability, and thus P is set to 0.15% or less. Particularly, when the hole expandability and the weldability are considered, P is desirably 0.02% or less. Incidentally, it is difficult to set P to 0% in terms of operation, and thus 0% is not included.

## S: 0.03% or less

S is an impurity contained in molten iron, and is an element that not only causes cracking at the time of hot rolling but also generates an A-based inclusion deteriorating the hole expandability. For this reason, S should be decreased as much as possible, but as long as S is 0.03% or less, it falls within an allowable range, and thus S is set to 0.03% or less. However, when the hole expandability to such extent is needed, S is preferably 0.01% or less, and is more preferably 0.005% or less. Incidentally, it is difficult to set S to 0% in terms of operation, and thus 0% is not included.

## Al: 0.001 to 2%

For molten steel deoxidation in a refining process of the steel, 0.001% or more of Al is added, but the upper limit is set to 2% because an increase in cost is caused. When Al is added in large amounts, the content of non-metal inclusions is increased and the ductility and the toughness deteriorate, and thus Al is desirably 0.06% or less. It is further desirably 0.04% or less.

Al is an element having a function of suppressing precipitation of iron-based carbide such as cementite in the structure, similarly to Si. For obtaining this function effect, Al is desirably 0.016% or more. It is further desirably 0.016 to 0.04%.

## N: 0.01% or less

N is an element that should be decreased as much as possible, but as long as N is 0.01% or less, it falls within an allowable range. In terms of aging resistance, however, N is desirably 0.005% or less. Incidentally, it is difficult to set N to 0% in terms of operation, and thus 0% is not included.

The present invention hot-rolled steel sheet may also contain one type or two or more types of Ti, Nb, Cu, Ni, Mo, V, and Cr according to need. The present invention hot-rolled steel sheet may also further contain one type or two or more types of Mg, Ca, and REM.

Hereinafter, there will be explained reasons for limiting chemical compositions of the above-described elements.

Ti, Nb, Cu, Ni, Mo, V, and Cr each are an element improving the strength by precipitation strengthening or solid-solution strengthening, and one type or two or more types of these elements may also be added.

However, when Ti is less than 0.015%, Nb is less than 0.005%, Cu is less than 0.02%, Ni is less than 0.01%, Mo is less than 0.01%, V is less than 0.01%, and Cr is less than 0.01%, their addition effects cannot be obtained sufficiently.

On the other hand, when Ti is greater than 0.18%, Nb is greater than 0.06%, Cu is greater than 1.2%, Ni is greater than 0.6%, Mo is greater than 1%, V is greater than 0.2%, and Cr is greater than 2%, the addition effects are saturated and economic efficiency decreases. Therefore, it is desirable that Ti is 0.015 to 0.18%, Nb is 0.005 to 0.6%, Cu is 0.02 to 1.2%, Ni is 0.01 to 0.6%, Mo is 0.01 to 1%, V is 0.01 to 0.2%, and Cr is 0.01 to 2%.

Mg, Ca, and REM (rare-earth element) each are an element that controls the form of non-metal inclusions to be the starting point of fracture to cause the deterioration of the workability and improves the workability, and one type or two or more types of these elements may also be added. When Mg, Ca, and REM are each less than 0.0005%, their addition effects are not exhibited.

## 12

On the other hand, when Mg is greater than 0.01%, Ca is greater than 0.01%, and REM is greater than 0.1%, the addition effects are saturated and economic efficiency decreases. Therefore, it is desirable that Mg is 0.0005 to 0.01%, Ca is 0.0005 to 0.01%, and REM is 0.0005 to 0.1%.

Incidentally, the present invention hot-rolled steel sheet may also contain 1% or less in total of one type or two or more types of Zr, Sn, Co, Zn, and W within a range that does not impair the characteristics of the present invention hot-rolled steel sheet. However, Sn is desirably 0.05% or less in order to suppress occurrence of a flaw at the time of hot rolling.

## B: 0.0002 to 0.002%

B is an element that increases the hardenability and increases a structural fraction of the low-temperature transformation generating phase being a hard phase and thus is added according to need. When B is less than 0.0002%, its addition effect cannot be obtained, and when B exceeds 0.002%, on the other hand, the addition effect is saturated, and further there is a risk that the recrystallization of austenite in hot rolling is suppressed and the  $\gamma$  to  $\alpha$  transformation texture from non-recrystallized austenite is strengthened to deteriorate the isotropy. Therefore, B is set to 0.0002 to 0.002%.

Further, B is also an element causing slab cracking in a cooling process after continuous casting, and from this viewpoint, is desirably 0.0015% or less. It is desirably 0.001 to 0.0015%.

## 30 (Microstructure)

Next, there will be explained metallurgical factors such as a microstructure of the present invention hot-rolled steel sheet in detail.

The microstructure of the present invention hot-rolled steel sheet is composed of 35% or less in a structural fraction of pro-eutectoid ferrite and a balance of the low-temperature transformation generating phase. The low-temperature transformation generating phase means a continuous cooling transformation structure, and is a structure recognized as bainite in general.

Generally, steel sheets having the same tensile strength are compared, and then where a microstructure is an uniform structure occupied by a structure such as the continuous cooling transformation structure, the microstructure shows a tendency to be excellent in local elongation as is typified by a hole expanding value, for example. Where the microstructure is a composite structure composed of pro-eutectoid ferrite being a soft phase and a hard low-temperature transformation generating phase (continuous cooling transformation structure, including martensite in MA), the microstructure shows a tendency to be excellent in uniform elongation that is typified by a work hardening coefficient  $n$  value.

In the present invention hot-rolled steel sheet, the microstructure is designed to be the composite structure composed of 35% or less in a structural fraction of pro-eutectoid ferrite and a balance of the low-temperature transformation generating phase in order to ultimately balance the local elongation as is typified by the bendability and the uniform elongation.

When pro-eutectoid ferrite is greater than 35%, the bendability being an index of the local elongation decreases significantly, but the uniform elongation is not so improved, and thus the balance between the local elongation and the uniform elongation deteriorates. The lower limit of the structural fraction of pro-eutectoid ferrite is not limited in particular, but when the structural fraction is 5% or less, a

## 13

decrease in the uniform elongation becomes significant, and thus the structural fraction of pro-eutectoid ferrite is preferably greater than 5%.

The continuous cooling transformation structure (Zw) (low-temperature transformation generating phase) of the present invention hot-rolled steel sheet is a microstructure defined as a transformation structure positioned in the middle of a microstructure containing polygonal ferrite and pearlite to be generated by a diffusive mechanism and martensite to be generated by a non-diffusive shearing mechanism, as is described in The Iron and Steel Institute of Japan, Society of basic research, Bainite Research Committee/Edition; Recent Research on Bainitic Microstructures and Transformation Behavior of Low Carbon Steels—Final Report of Bainite Research Committee (in 1994, The Iron and Steel Institute of Japan) (“reference literature”).

That is, the continuous cooling transformation structure (Zw) (low-temperature transformation generating phase) is defined as a microstructure mainly composed of Bainitic ferrite ( $\alpha_B^o$ ), Granular bainitic ferrite ( $\alpha_B$ ), and Quasi-polygonal ferrite ( $\alpha_q$ ), and further containing a small amount of retained austenite ( $\gamma_r$ ) and Martensite-austenite (MA) as is described in the above-described reference literature on pages 125 to 127 as an optical microscopic observation structure.

Incidentally, similarly to polygonal ferrite (PF), an internal structure of  $\alpha_q$  does not appear by etching, but a shape of  $\alpha_q$  is acicular, and it is definitely distinguished from PF. Here, of a targeted crystal grain, a peripheral length is set to  $lq$  and a circle-equivalent diameter is set to  $dq$ , and then a grain having a ratio ( $lq/dq$ ) satisfying  $lq/dq \geq 3.5$  is  $\alpha_q$ .

The continuous cooling transformation structure (Zw) (low-temperature transformation generating phase) of the present invention hot-rolled steel sheet is a microstructure containing one type or two or more types of  $\alpha_B^o$ ,  $\alpha_B$ , and  $\alpha_q$ . Further, the continuous cooling transformation structure (Zw) (low-temperature transformation generating phase) of the present invention hot-rolled steel sheet may also further contain one of a small amount of  $\gamma_r$  and MA, or both of them, in addition to one type or two or more types of  $\alpha_B^o$ ,  $\alpha_B$ , and  $\alpha_q$ . Incidentally, the total content of  $\gamma_r$  and MA is set to 3% or less in a structural fraction.

There is sometimes a case that the continuous cooling transformation structure (Zw) (low-temperature transformation generating phase) is not easily discerned by observation by optical microscope in etching using a nital reagent. In such a case, it is discerned by using the EBSP-OIM<sup>TM</sup>. The EBSP-OIM<sup>TM</sup> (Electron Back Scatter Diffraction Pattern-Orientation Image Microscopy) method is constituted by a device and software in which a highly inclined sample in a scanning electron microscope (Scanning Electron Microscope) is irradiated with electron beams, a Kikuchi pattern formed by backscattering is photographed by a high-sensitive camera and is image processed by a computer, and thereby a crystal orientation at an irradiation point is measured for a short time period.

In the EBSP method, it is possible to quantitatively analyze a microstructure and a crystal orientation of a bulk sample surface. As long as an area to be analyzed by the EBSP method is within an area capable of being observed by the SEM, it is possible to analyze the area with a minimum resolution of 20 nm, depending on the resolution of the SEM.

The analysis by the EBSP-OIM<sup>TM</sup> method is performed by mapping an area to be analyzed to tens of thousands of equally-spaced grid points. It is possible to see crystal orientation distributions and sizes of crystal grains within

## 14

the sample in a polycrystalline material. In the present invention hot-rolled steel sheet, one discernible from a mapped image with an orientation difference between packets defined as 15° may also be defined as a grain diameter of the continuous cooling transformation structure (Zw) (low-temperature transformation generating phase) for convenience. In this case, a large angle tilt grain boundary having a crystal orientation difference of 15° or more is defined as a grain boundary.

5 Further, the structural fraction of pro-eutectoid ferrite was obtained by a Kernel Average Misorientation (KAM) method being equipped with the EBSP-OIM<sup>TM</sup>. The KAM method is that a calculation, in which orientation differences among pixels of first approximations being adjacent six 15 pixels of a certain regular hexagon of measurement data, or second approximations being 12 pixels positioned outside the six pixels, or third approximations being 18 pixels positioned further outside the 12 pixels are averaged and an obtained value is set to a value of the center pixel, is 20 performed with respect to each pixel.

This calculation is performed so as not to exceed a grain boundary, thereby making it possible to create a map representing an orientation change within a grain. That is, this map represents a distribution of strain based on a local 25 orientation change within a grain. Note that in the analysis, the condition of which in the EBSP-OIM<sup>TM</sup>, the orientation difference among adjacent pixels is calculated is set to the third approximation and one having this orientation difference being 5° or less is displayed.

30 In examples of the present invention, the condition of which in the EBSP-OIM (registered trademark), the orientation difference among adjacent pixels is calculated is set to the third approximation and this orientation difference is set to 5° or less, and the above-described orientation difference 35 third approximation is greater than 1°, which is defined as the continuous cooling transformation structure (Zw) (low-temperature transformation generating phase), and it is 1° or less, which is defined as ferrite. This is because polygonal pro-eutectoid ferrite transformed at high temperature is 40 generated in a diffusion transformation, and thus a dislocation density is small and strain within the grain is small, and thus, a difference within the grain in the crystal orientation is small, and according to the results of various examinations 45 that have been performed so far by the present inventors, a volume fraction of polygonal ferrite obtained by observation of optical microscope and an area fraction of an area obtained by 1° or less of the orientation difference third approximation measured by the KAM method substantially agree with each other.

## 50 (Manufacturing Method)

Next, there will be explained conditions of a manufacturing method of the present invention hot-rolled steel sheet, (which will be called a “present invention manufacturing method,” hereinafter).

55 The present inventors explored hot rolling conditions making austenite recrystallize sufficiently after finish rolling or during finish rolling in order to secure the isotropy but suppressing grain growth of recrystallized grains as much as possible and achieving the isotropy and the low-temperature toughness.

60 First, in the present invention manufacturing method, a manufacturing method of a steel billet to be performed prior to a hot rolling process is not particularly limited. That is, in the manufacturing method of the steel billet, subsequent to a melting process by a shaft furnace, a steel converter, an electric furnace, or the like, in various secondary refining processes, a component adjustment is performed so as to be

an aimed chemical composition. Next, a casting process may also be performed by normal continuous casting, or casting by an ingot method, or further a method such as thin slab casting.

Incidentally, a scrap may also be used for a raw material. Further, when a slab is obtained by continuous casting, the slab may be directly transferred to a hot rolling mill as it is in a high-temperature cast slab state, or it may also be cooled to a room temperature and then reheated in a heating furnace, and then hot rolled.

The slab obtained by the above-described manufacturing method is heated in a slab heating process prior to the hot rolling process, but in the present invention manufacturing method, a heating temperature is not determined in particular. However, when the heating temperature is higher than 1260° C., a yield decreases due to scale off, and thus the heating temperature is preferably 1260° C. or lower. On the other hand, when the heating temperature is lower than 1150° C., operational efficiency deteriorates significantly in terms of a schedule, and thus the heating temperature is desirably 1150° C. or higher.

Further, a heating time period in the slab heating process is not determined in particular, but in terms of avoiding central segregation and the like, after the temperature reaches a predetermined heating temperature, the heating temperature is desirably maintained for 30 minutes or longer. However, when the cast slab after being subjected to casting is directly transferred to a hot rolling mill as it is in a high-temperature cast slab state to be rolled, the heating time period is not limited to this.

(First Hot Rolling)

After the slab heating process, the slab extracted from the heating furnace is subjected to a rough rolling process being first hot rolling to be rough rolled without a wait, and thereby a rough bar is obtained.

The rough rolling process (first hot rolling) is performed at a temperature of not lower than 1000° C. nor higher than 1200° C. for reasons to be explained below. When a rough rolling finishing temperature is lower than 1000° C., reduction is performed in a state where the vicinity of a surface layer of the rough bar is in a non-recrystallization temperature region, the texture is developed, and the isotropy deteriorates. Further, hot deformation resistance in the rough rolling increases, to thereby cause a risk that an impediment is caused to the rough rolling operation.

On the other hand, when the rough rolling finishing temperature is higher than 1200° C., the average crystal grain diameter is increased to decrease the toughness. Further, a secondary scale to be generated during the rough rolling grows too much, to thereby make it difficult to remove the scale in descaling or finish rolling to be performed later. When the rough rolling finishing temperature is higher than 1150° C., there is sometimes a case that inclusions are drawn and the hole expandability deteriorates, and thus it is desirably 1150° C. or lower.

Further, in the rough rolling process (first hot rolling), in a temperature range of not lower than 1000° C. nor higher than 1200° C., rolling at a reduction ratio of 40% or more is performed one time or more. When the reduction ratio in the rough rolling process is less than 40%, the average crystal grain diameter is increased and the toughness decreases. When the reduction ratio is 40% or more, the crystal grain diameter becomes uniform and small. On the other hand, when the reduction ratio is greater than 65%, there is sometimes a case that inclusions are drawn and the hole expandability deteriorates, and thus it is desirably 65% or less. Incidentally, in the rough rolling, when the reduction

ratio at a final stage and the reduction ratio at a stage prior to the final stage are less than 20%, the average crystal grain diameter is increased easily, and thus in the rough rolling, the reduction ratio at the final stage and the reduction ratio at the stage prior to the final stage are desirably 20% or more.

Incidentally, in terms of decreasing the average crystal grain diameter of a final product, an austenite grain diameter after the rough rolling, namely before the finish rolling is 10 important and the austenite grain diameter before the finish rolling is desirably small.

As long as the austenite grain diameter before the finish rolling is 200  $\mu\text{m}$  or less, it is possible to greatly promote grain refining and homogenizing. For efficiently obtaining 15 this promoting effect, the austenite grain diameter is desirably set to 100  $\mu\text{m}$  or less. In order to achieve it, the rolling at a reduction ratio of 40% or more is desirably performed two or more times in the rough rolling process. However, when in the rough rolling process, the rolling is performed 20 greater than 10 times, there is a concern that the temperature decreases or a scale is generated excessively.

In this manner, the austenite grain diameter before the finish rolling is decreased, which is effective for promoting the recrystallization of austenite in the finish rolling later. It 25 is supposed that this is because an austenite grain boundary after the rough rolling (namely before the finish rolling) functions as one of recrystallization nuclei during the finish rolling.

The austenite grain diameter after the rough rolling is 30 measured as follows. That is, the steel billet (rough bar) after the rough rolling (before being subjected to the finish rolling) is quenched as much as possible, and is desirably cooled at a cooling rate of 10° C./second or more. The structure of a cross section of the cooled steel billet is etched 35 to make the austenite grain boundaries appear, and the austenite grain boundaries are measured by an optical microscope. On this occasion, at 50 magnifications or more, 20 visual fields or more are measured by image analysis or a point counting method.

40 The rough bars obtained after the completion of the rough rolling process may also be joined between the rough rolling process and a finish rolling process to then have endless rolling such that the finish rolling process is performed continuously performed thereon. On this occasion, the rough 45 bars may also be coiled into a coil shape once, stored in a cover having a heat insulating function according to need, and uncoiled again to be joined.

On the occasion of the hot rolling process, temperature variations of the rough bar in a rolling direction, in a sheet 50 width direction, and in a sheet thickness direction are desirably controlled to be small. In this case, according to need, a heating apparatus capable of controlling the temperature variations of the rough bar in the rolling direction, in the sheet width direction, and in the sheet thickness 55 direction may be disposed between a roughing mill in the rough rolling process and a finishing mill in the finish rolling process, or between respective stands in the finish rolling process, and thereby the rough bar may be heated.

As a system of the heating apparatus, various heating 60 systems such as gas heating, electrical heating, and induction heating are conceivable, but as long as the heating system makes it possible to control the temperature variations of the rough bar in the rolling direction, in the sheet width direction, and in the sheet thickness direction to be small, any one of well-known systems may also be used.

Incidentally, as the system of the heating apparatus, an induction heating system having an industrially good tem-

perature control response is preferred. If among various induction heating systems, a plurality of transverse-type induction heating apparatuses capable of being shifted in the sheet width direction is installed, a temperature distribution in the sheet width direction can be arbitrarily controlled according to the sheet width, and thus the transverse-type induction heating apparatuses are more preferred. Further, as the system of the heating apparatus, a heating apparatus constituted by the combination of a transverse-type induction heating apparatus and a solenoid-type induction heating apparatus that excels in heating across the entire sheet width is the most preferred.

When the temperature is controlled using these heating apparatuses, it sometimes becomes necessary to control an amount of heating by the heating apparatus. In this case, the internal temperature of the rough bar cannot be measured actually, and thus previously measured actual data such as a charged slab temperature, a slab furnace existing time period, a heating furnace atmospheric temperature, a heating furnace extraction temperature, and further a table roller transfer time period are used to estimate temperature distributions in the rolling direction, in the sheet width direction, and in the sheet thickness direction when the rough bar reaches the heating apparatus, and then the amount of heating by the heating apparatus is desirably controlled.

Incidentally, the control of the amount of heating by the induction heating apparatus is controlled in the following manner, for example. A characteristic of the induction heating apparatus (transverse-type induction heating apparatus) is that when an alternating current is applied to a coil, a magnetic field is generated in its inside. In an electric conductor positioned in the magnetic field, an eddy current having an orientation opposite to the current in the coil occurs in a circumferential direction perpendicular to a magnetic flux by an electromagnetic induction effect, and by Joule heat of the eddy current, the electric conductor is heated.

The eddy current occurs most strongly on the inner surface of the coil and decreases exponentially toward the inside (this phenomenon is called a skin effect). Thus, as a frequency is smaller, a current penetration depth is increased and a heating pattern uniform in the thickness direction is obtained, and conversely, as a frequency is larger, the current penetration depth is decreased and a heating pattern that exhibits its peak at a surface layer and has small overheating is obtained in the thickness direction.

Therefore, by the transverse-type induction heating apparatus, the heating of the rough bar in the rolling direction and in the sheet width direction can be performed in a conventional manner, and further in terms of the heating in the sheet thickness direction, by changing the frequency of the transverse-type induction heating apparatus, the penetration depth is varied and the heating temperature pattern in the sheet thickness direction is controlled, to thereby make it possible to achieve uniformity of the temperature distributions. Incidentally, a frequency-changeable-type induction heating apparatus is preferably used in this case, but the frequency may also be changed by adjusting a capacitor.

With regard to the control of the amount of heating by the induction heating apparatus, a plurality of inductors having different frequencies may be disposed and an allocation of an amount of heating by each of the inductors may be changed so as to obtain the necessary heating pattern in the thickness direction. With regard to the control of the amount of heating by the induction heating apparatus, an air gap to a material to be heated is changed and thereby the frequency

changes, and thus by changing the air gap, the desired frequency and heating pattern may also be obtained.

A maximum height  $R_y$  of the steel sheet surface (rough bar surface) after the finish rolling is desirably  $15 \mu\text{m}$  ( $15 \mu\text{m}$   $R_y$ ,  $12.5 \text{ mm}$ ,  $\ln 12.5 \text{ mm}$ ) or less. This is clear because the fatigue strength of the hot-rolled or pickled steel sheet is correlated to the maximum height  $R_y$  of the steel sheet surface as is also described in Metal Material Fatigue Design Handbook, edited by The Society of Materials Science, Japan, on page 84, for example.

In order to obtain this surface roughness, a condition of an impact pressure  $P_{xa}$  flow rate  $L \geq 0.003$  of a high-pressure water onto the steel sheet surface is desirably satisfied in descaling. Further, the subsequent finish rolling is desirably performed within five seconds in order to prevent a scale from being generated again after the descaling.

#### (Second Hot Rolling)

After the rough rolling process (first hot rolling) is completed, the finish rolling process being second hot rolling is started. The time between the completion of the rough rolling process and the start of the finish rolling process is desirably set to 150 seconds or shorter. When the time between the completion of the rough rolling process and the start of the finish rolling process is longer than 150 seconds, the average crystal grain diameter is increased to cause the decrease in  $vTrs$ .

In the finish rolling process (second hot rolling), a finish rolling start temperature is set to  $1000^\circ\text{C}$ . or higher. When the finish rolling start temperature is lower than  $1000^\circ\text{C}$ ., at each finish rolling pass, the temperature of the rolling to be applied to the rough bar to be rolled is decreased, the reduction is performed in a non-recrystallization temperature region, the texture develops, and thus the isotropy deteriorates.

Incidentally, the upper limit of the finish rolling start temperature is not limited in particular. However, when it is  $1150^\circ\text{C}$ . or higher, a blister to be the starting point of a scaly spindle-shaped scale defect is likely to occur between a steel sheet base iron and a surface scale before the finish rolling and between passes, and thus the finish rolling start temperature is desirably lower than  $1150^\circ\text{C}$ .

In the finish rolling, a temperature determined by the chemical composition of the steel sheet is set to  $T_1$ , and in a temperature region of not lower than  $T_1+30^\circ\text{C}$ . nor higher than  $T_1+200^\circ\text{C}$ ., the rolling at 30% or more is performed in one pass at least one time. Further, in the finish rolling, the total of the reduction ratios is set to 50% or more.

Here,  $T_1$  is the temperature calculated by Expression (1) below.

$$T_1(\text{ }^\circ\text{C}) = 850 + 10 \times (C + N) \times Mn + 350 \times Nb + 250 \times Ti + 40 \times Cr + 100 \times Mo + 100 \times V \quad (1)$$

$C$ ,  $N$ ,  $Mn$ ,  $Nb$ ,  $Ti$ ,  $B$ ,  $Cr$ ,  $Mo$ , and  $V$  each represent the content of the element (mass %).

$T_1$  itself is obtained empirically. The present inventors learned empirically by experiments that the recrystallization in an austenite region of each steel is promoted on the basis of  $T_1$ .

When the total reduction ratio in the temperature region of not lower than  $T_1+30^\circ\text{C}$ . nor higher than  $T_1+200^\circ\text{C}$ . is less than 50%, rolling strain to be accumulated during the hot rolling is not sufficient and the recrystallization of austenite does not advance sufficiently. Therefore, the texture develops and the isotropy deteriorates. When the total reduction ratio is 70% or more, the sufficient isotropy can be obtained even though variations ascribable to temperature fluctuation or the like are considered. On the other hand, when the total

reduction ratio exceeds 90%, it becomes difficult to obtain the temperature region of  $T_1+200^\circ\text{ C.}$  or lower due to heat generation by working, and further a rolling load increases to cause a risk that the rolling becomes difficult to be performed.

In the finish rolling, in order to promote the uniform recrystallization caused by releasing the accumulated strain, the rolling at 30% or more is performed in one pass at least one time at not lower than  $T_1+30^\circ\text{ C.}$  nor higher than  $T_1+200^\circ\text{ C.}$

Incidentally, in order to promote the uniform recrystallization, it is necessary to suppress a working amount in a temperature region of lower than  $T_1+30^\circ\text{ C.}$  as small as possible. In order to achieve it, the reduction ratio at lower than  $T_1+30^\circ\text{ C.}$  is desirably 30% or less. In terms of sheet thickness accuracy and sheet shape, 10% or less of the reduction ratio is desirable. When the isotropy is further obtained, the reduction ratio in the temperature region of lower than  $T_1+30^\circ\text{ C.}$  is desirably 0%.

The finish rolling is desirably finished at  $T_1+30^\circ\text{ C.}$  or higher. In the hot rolling at lower than  $T_1+30^\circ\text{ C.}$ , the granulated austenite grains that are recrystallized once are elongated, thereby causing a risk that the isotropy deteriorates.

#### (Primary Cooling)

In the finish rolling, after the final reduction at a reduction ratio of 30% or more is performed, primary cooling is started in such a manner that a waiting time period  $t$  second satisfies Expression (2) below.

$$t \leq 2.5 \times t_1 \quad (2)$$

Here,  $t_1$  is obtained by Expression (3) below.

$$t_1 = 0.001 \times ((T_f - T_1) \times P_1 / 100)^2 - 0.109 \times ((T_f - T_1) \times P_1 / 100) + 3.1 \quad (3)$$

Here, in Expression (3) above,  $T_f$  represents the temperature of the steel billet obtained after the final reduction at a reduction ratio of 30% or more, and  $P_1$  represents the reduction ratio of the final reduction at 30% or more.

Incidentally, the “final reduction at a reduction ratio of 30% or more” indicates the rolling performed finally among the rollings whose reduction ratio becomes 30% or more out of the rollings in a plurality of passes performed in the finish rolling. For example, when among the rollings in a plurality of passes performed in the finish rolling, the reduction ratio of the rolling performed at the final stage is 30% or more, the rolling performed at the final stage is the “final reduction at a reduction ratio of 30% or more.” Further, when among the rollings in a plurality of passes performed in the finish rolling, the reduction ratio of the rolling performed prior to the final stage is 30% or more and after the rolling performed prior to the final stage (rolling at a reduction ratio of 30% or more) is performed, the rolling whose reduction ratio becomes 30% or more is not performed, the rolling performed prior to the final stage (rolling at a reduction ratio of 30% or more) is the “final reduction at a reduction ratio of 30% or more.”

In the finish rolling, the waiting time period  $t$  second until the primary cooling is started after the final reduction at a reduction ratio of 30% or more is performed greatly affects the austenite grain diameter. That is, it greatly affects an equiaxed grain fraction and a coarse grain area ratio of the steel sheet.

When the waiting time period  $t$  second exceeds  $t_1 \times 2.5$ , the recrystallization is already almost completed, but the crystal grains grow significantly and grain coarsening advances, and thereby the  $r$  value and the elongation are decreased.

The waiting time period  $t$  second further satisfies Expression (4) below, thereby making it possible to preferentially suppress the growth of the crystal grains. Consequently, even though the recrystallization does not advance sufficiently, it is possible to sufficiently improve the elongation of the steel sheet and to improve the fatigue property simultaneously.

$$t < t_1 \quad (4)$$

10 At the same time, the waiting time period  $t$  second further satisfies Expression (5) below, and thereby the recrystallization advances sufficiently and the crystal orientations are randomized. Therefore, it is possible to sufficiently improve the elongation of the steel sheet and to greatly improve the 15 isotropy simultaneously.

$$t_1 \leq t \leq t_1 \times 2.5 \quad (5)$$

The waiting time period  $t$  second satisfies Expression (5) above, and thereby the average value of the pole densities of 20 the  $\{100\} < 011 >$  to  $\{223\} < 110 >$  orientation group shown in FIG. 1 becomes 2.0 or less and the pole density of the  $\{332\} < 113 >$  crystal orientation shown in FIG. 2 becomes 3.0 or less. Consequently, the isotropic index becomes 6.0 or more and the sheet thickness uniformity and circularity that 25 sufficiently satisfy the part property in a state where the steel sheet remains worked are achieved.

Here, as shown in FIG. 4, on a continuous hot rolling line 1, the steel billet (slab) heated to a predetermined temperature in the heating furnace is rolled in a roughing mill 2 and in a finishing mill 3 sequentially to be a hot-rolled steel sheet 4 having a predetermined thickness, and the hot-rolled steel sheet 4 is carried out onto a run-out-table 5. In the present invention manufacturing method, in the rough rolling process (first hot rolling) performed in the roughing mill 2, the 30 rolling at a reduction ratio of 40% or more is performed on the steel billet (slab) one time or more in the temperature range of not lower than  $1000^\circ\text{ C.}$  nor higher than  $1200^\circ\text{ C.}$

The rough bar rolled to a predetermined thickness in the roughing mill 2 in this manner is next finish rolled (is 35 subjected to the second hot rolling) through a plurality of rolling stands 6 of the finishing mill 3 to be the hot-rolled steel sheet 4. Then, in the finishing mill 3, the rolling at 30% or more is performed in one pass at least one time in the temperature region of not lower than the temperature  $T_1+30^\circ\text{ C.}$  nor higher than  $T_1+200^\circ\text{ C.}$  Further, in the 40 finishing mill 3, the total of the reduction ratios becomes 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 915

Expressions (4) and (5) above is sometimes caused. In such a case, the primary cooling is started by the inter-stand cooling nozzles 10 disposed between the respective the rolling stands 6 of the finishing mill 3.

Further, for example, when the final reduction at a reduction ratio of 30% or more is performed at the rolling stand 6 disposed at the rear stage of the finishing mill 3 (on the right side in FIG. 4, on the downstream side of the rolling), even though the start of the primary cooling is performed by the cooling nozzles 11 disposed in the run-out-table 5, there is sometimes a case that the waiting time period  $t$  second can satisfy Expression (2) above or Expressions (4) and (5) above. In such a case, the primary cooling may also be started by the cooling nozzles 11 disposed in the run-out-table 5. Needless to say, as long as the performance of the final reduction at a reduction ratio of 30% or more is completed, the primary cooling may also be started by the inter-stand cooling nozzles 10 disposed between the respective the rolling stands 6 of the finishing mill 3.

Then, in this primary cooling, the cooling that at an average cooling rate of 50° C./second or more, a temperature change (temperature drop) becomes not lower than 40° C. nor higher than 140° C. is performed.

When the temperature change is lower than 40° C., the recrystallized austenite grains grow and the low-temperature toughness deteriorates. The temperature change is set to 40° C. or higher, thereby making it possible to suppress coarsening of the austenite grains. When the temperature change is lower than 40° C., the effect cannot be obtained. On the other hand, when the temperature change exceeds 140° C., the recrystallization becomes insufficient to make it difficult to obtain a targeted random texture. Further, a ferrite phase effective for the elongation is also not obtained easily and the hardness of a ferrite phase becomes high, and thereby the elongation and local ductility also deteriorate. Further, when the temperature change is higher than 140° C., an overshoot to/beyond an Ar3 transformation point temperature is likely to be caused. In the case, even by the transformation from recrystallized austenite, as a result of sharpening variant selection, the texture is formed and the isotropy decreases consequently.

When the average cooling rate in the primary cooling is less than 50° C./second, as expected, the recrystallized austenite grains grow and the low-temperature toughness deteriorates. The upper limit of the average cooling rate is not determined in particular, but in terms of the steel sheet shape, 200° C./second or less is considered to be proper.

Further, in order to suppress the grain growth and obtain the more excellent low-temperature toughness, a cooling device between passes or the like is desirably used to bring the heat generation by working between the respective stands of the finish rolling to 18° C. or lower.

A rolling ratio (the reduction ratio) can be obtained by actual performances or calculation from the rolling load, sheet thickness measurement, or/and the like. The temperature of the steel billet during the rolling can be obtained by actual measurement by a thermometer being disposed between the stands, or can be obtained by simulation by considering the heat generation by working from a line speed, the reduction ratio, or/and like, or can be obtained by the both methods.

Further, as has been explained previously, in order to promote the uniform recrystallization, the working amount in the temperature region of lower than T1+30° C. is desirably as small as possible and the reduction ratio in the temperature region of lower than T1+30° C. is desirably 30% or less. For example, in the event that in the finishing

mill 3 on the continuous hot rolling line 1 shown in FIG. 4, in passing through one or two or more of the rolling stands 6 disposed on the front stage side (on the left side in FIG. 4, on the upstream side of the rolling), the steel sheet is in the temperature region of not lower than T1+30° C. nor higher than T1+200° C., and in passing through one or two or more of the rolling stands 6 disposed on the subsequent rear stage side (on the right side in FIG. 4, on the downstream side of the rolling), the steel sheet is in the temperature region of lower than T1+30° C., when the steel sheet passes through one or two or more of the rolling stands 6 disposed on the subsequent rear stage side (on the right side in FIG. 4, on the downstream side of the rolling), even though the reduction is not performed or is performed, the reduction ratio at lower than T1+30° C. is desirably 30% or less in total. In terms of the sheet thickness accuracy and the sheet shape, the reduction ratio at lower than T1+30° C. is desirably a reduction ratio of 10% or less in total. When the isotropy is further obtained, the reduction ratio in the temperature region of lower than T1+30° C. is desirably 0%.

In the present invention manufacturing method, a rolling speed is not limited in particular. However, when the rolling speed on the final stand side of the finish rolling is less than 400 mpm,  $\gamma$  grains grow to be coarse, regions in which ferrite can precipitate for obtaining the ductility are decreased, and thus the ductility is likely to deteriorate. Even though the upper limit of the rolling speed is not limited in particular, the effect of the present invention can be obtained, but it is actual that the rolling speed is 1800 mpm or less due to facility restriction. Therefore, in the finish rolling process, the rolling speed is desirably not less than 400 mpm nor more than 1800 mpm.

Further, within three seconds after the completion of the primary cooling, secondary cooling in which cooling is performed at an average cooling rate of 15° C./second or more is performed. When the time period to the start of the secondary cooling exceeds three seconds, pearlite transformation occurs and the targeted microstructure cannot be obtained.

When the average cooling rate of the secondary cooling is less than 15° C./second, as expected, the pearlite transformation occurs and the targeted microstructure cannot be obtained. Even though the upper limit of the average cooling rate of the secondary cooling is not limited in particular, the effect of the present invention can be obtained, but when warpage of the steel sheet due to thermal strain is considered, the average cooling rate is desirably 300° C./second or less.

The average cooling rate is not less than 15° C./second nor more than 50° C./second, which is a region allowing stable manufacturing. Further, as will be shown in examples, the region of 30° C./second or less is a region allowing more stable manufacturing.

Next, air cooling is performed for 1 to 20 seconds in a temperature region of lower than the Ar3 transformation point temperature and an Ar1 transformation point temperature or higher. This air cooling is performed in the temperature region of lower than the Ar3 transformation point temperature and the Ar1 transformation point temperature or higher (a ferrite-austenite-two-phase temperature region) in order to promote the ferrite transformation. When the air cooling is performed for less than one second, the ferrite transformation in the two-phase region is not sufficient and thus the sufficient uniform elongation cannot be obtained, and when the air cooling is performed for greater than 20 seconds, on the other hand, the pearlite transformation occurs and the targeted microstructure cannot be obtained.

The temperature region where the air cooling is performed for 1 to 20 seconds is desirably not lower than the Ar1 transformation point temperature nor higher than 860°C. in order to easily promote the ferrite transformation. A holding time period (an air cooling time period) for 1 to 20 seconds is desirably for 1 to 10 seconds in order not to decrease the productivity extremely.

The Ar3 transformation point temperature can be easily calculated by the following calculation expression (a relational expression with the chemical composition), for example. When the Si content (mass %) is set to [Si], the Cr content (mass %) is set to [Cr], the Cu content (mass %) is set to [Cu], the Mo content (mass %) is set to [Mo], and the Ni content (mass %) is set to [Ni], the Ar3 transformation point temperature can be defined by Expression (6) below.

$$Ar3 = 910 - 310 \times [C] + 25 \times [Si] - 80 \times [Mneq] \quad (6)$$

When B is not added, [Mneq] is defined by Expression (7) below.

$$[Mneq] = [Mn] + [Cr] + [Cu] + [Mo] + ([Ni]/2) + 10([Nb] - 0.02) \quad (7)$$

When B is added, [Mneq] is defined by Expression (8) below.

$$[Mneq] = [Mn] + [Cr] + [Cu] + [Mo] + ([Ni]/2) + 10([Nb] - 0.02) + 1 \quad (8)$$

Subsequently, in a coiling process, a coiling temperature is set to not lower than 450°C. nor higher than 550°C. When the coiling temperature is higher than 550°C., after the coiling, tempering in a hard phase occurs and the strength decreases. On the other hand, when the coiling temperature is lower than 450°C., during cooling after the coiling, non-transformed austenite is stabilized, and in a product steel sheet, retained austenite is contained and martensite is generated, and thereby the hole expandability decreases.

Incidentally, with the aim of achieving the improvement of the ductility by correction of the steel sheet shape and/or introduction of mobile dislocation, skin pass rolling at a reduction ratio of not less than 0.1% nor more than 2% is desirably performed after the completion of all the processes.

Further, after the completion of all the processes, pickling may also be performed with the aim of removing the scale adhering to the surface of the obtained hot-rolled steel sheet.

After the pickling, on the hot-rolled steel sheet, skin pass or cold rolling at a reduction ratio of 10% or less may also be performed inline or offline.

On the present invention hot-rolled steel sheet, a heat treatment may also be performed on a hot dipping line after the casting, after the hot rolling, or after the cooling, and further on the heat-treated hot-rolled steel sheet, a surface treatment may also be performed separately. On the hot dipping line, plating is performed, and thereby the corrosion resistance of the hot-rolled steel sheet is improved.

When galvanizing is performed on the pickled hot-rolled steel sheet, after the hot-rolled steel sheet is dipped in a galvanizing bath to then be pulled up, an alloying treatment may also be performed on the hot-rolled steel sheet according to need. By performing the alloying treatment, in addition to the improvement of the corrosion resistance, welding resistance against various weldings such as spot welding is improved.

## EXAMPLE

Next, examples of the present invention will be explained, but conditions of the examples are condition examples employed for confirming the applicability and effects of the present invention, and the present invention is not limited to these condition examples. The present invention can employ various conditions as long as the object of the present invention is achieved without departing from the spirit of the invention.

### Example 1

Cast billets A to P having chemical compositions shown in Table 1 were each melted in a steel converter in a secondary refining process to be subjected to continuous casting and then were directly transferred or reheated to be subjected to rough rolling. In the subsequent finish rolling, they were each reduced to a sheet thickness of 2.0 to 3.6 mm and were subjected to cooling by inter-stand cooling of a finishing mill or on a run-out-table and then were coiled, and hot-rolled steel sheets were manufactured. Manufacturing conditions are shown in Table 2.

Incidentally, the balance of the chemical composition shown in Table 1 is composed of Fe and inevitable impurities, and each underline in Table 1 and Table 2 indicates that the value is outside the range of the present invention or outside the preferable range of the present invention.

TABLE 1

| STEEL | CHEMICAL COMPOSITION (UNIT: MASS %) |      |      |       |       |       |        |       |       |      |      |      |
|-------|-------------------------------------|------|------|-------|-------|-------|--------|-------|-------|------|------|------|
|       | C                                   | Si   | Mn   | P     | S     | Al    | N      | Ti    | Nb    | Cu   | Ni   | Mo   |
| A     | 0.070                               | 1.20 | 2.51 | 0.016 | 0.003 | 0.023 | 0.0026 | 0.144 | 0.020 | 0.00 | 0.00 | 0.00 |
| B     | 0.071                               | 1.17 | 2.46 | 0.011 | 0.002 | 0.029 | 0.0040 | 0.179 | 0.017 | 0.00 | 0.00 | 0.00 |
| C     | <u>0.067</u>                        | 0.14 | 1.98 | 0.007 | 0.001 | 0.011 | 0.0046 | 0.091 | 0.038 | 0.00 | 0.00 | 0.00 |
| D     | <u>0.036</u>                        | 0.94 | 1.34 | 0.008 | 0.001 | 0.020 | 0.0028 | 0.126 | 0.041 | 0.00 | 0.00 | 0.00 |
| E     | <u>0.043</u>                        | 0.98 | 0.98 | 0.010 | 0.001 | 0.036 | 0.0034 | 0.099 | 0.000 | 0.00 | 0.00 | 0.00 |
| F     | <u>0.042</u>                        | 0.73 | 1.04 | 0.011 | 0.001 | 0.024 | 0.0041 | 0.035 | 0.019 | 0.00 | 0.00 | 0.00 |
| G     | 0.089                               | 0.91 | 1.20 | 0.008 | 0.001 | 0.033 | 0.0038 | 0.000 | 0.000 | 0.00 | 0.00 | 0.00 |
| H     | 0.180                               | 0.03 | 0.72 | 0.017 | 0.004 | 0.011 | 0.0035 | 0.025 | 0.000 | 0.00 | 0.00 | 0.00 |
| I     | <u>0.022</u>                        | 0.05 | 1.12 | 0.009 | 0.004 | 0.025 | 0.0047 | 0.102 | 0.000 | 0.00 | 0.00 | 0.00 |
| J     | 0.004                               | 0.12 | 1.61 | 0.080 | 0.002 | 0.041 | 0.0027 | 0.025 | 0.025 | 0.00 | 0.00 | 0.00 |
| K     | <u>0.230</u>                        | 0.18 | 0.74 | 0.017 | 0.002 | 0.005 | 0.0051 | 0.000 | 0.000 | 0.00 | 0.00 | 0.00 |
| L     | 0.091                               | 0.02 | 1.50 | 0.007 | 0.001 | 0.011 | 0.0046 | 0.026 | 0.000 | 0.06 | 0.03 | 0.00 |
| M     | 0.100                               | 0.03 | 1.45 | 0.008 | 0.001 | 0.020 | 0.0028 | 0.020 | 0.000 | 0.00 | 0.03 | 0.00 |
| N     | 0.081                               | 0.01 | 1.51 | 0.010 | 0.001 | 0.036 | 0.0034 | 0.022 | 0.000 | 0.00 | 0.00 | 0.48 |
| O     | 0.090                               | 0.02 | 1.55 | 0.011 | 0.001 | 0.024 | 0.0041 | 0.024 | 0.011 | 0.00 | 0.00 | 0.00 |
| P     | 0.087                               | 0.02 | 1.52 | 0.008 | 0.001 | 0.033 | 0.0038 | 0.023 | 0.000 | 0.00 | 0.00 | 0.00 |
| Q     | 0.084                               | 0.02 | 1.49 | 0.007 | 0.001 | 0.031 | 0.0039 | 0.000 | 0.000 | 0.00 | 0.00 | 0.00 |

TABLE 1-continued

| STEEL | CHEMICAL COMPOSITION (UNIT: MASS %) |      |        |        |        |        |        | NOTE              |
|-------|-------------------------------------|------|--------|--------|--------|--------|--------|-------------------|
|       | V                                   | Cr   | B      | Mg     | Ca     | Rem    | OTHERS |                   |
| A     | 0.00                                | 0.00 | 0.0014 | 0.0022 | 0.0000 | 0.0000 | 0.0000 | PRESENT INVENTION |
| B     | 0.00                                | 0.00 | 0.0000 | 0.0000 | 0.0024 | 0.0000 | 0.0000 | PRESENT INVENTION |
| C     | 0.00                                | 0.00 | 0.0000 | 0.0019 | 0.0000 | 0.0000 | 0.0000 | COMPARATIVE STEEL |
| D     | 0.00                                | 0.00 | 0.0000 | 0.0000 | 0.0000 | 0.0000 | 0.0000 | COMPARATIVE STEEL |
| E     | 0.00                                | 0.00 | 0.0009 | 0.0000 | 0.0021 | 0.0000 | 0.0000 | COMPARATIVE STEEL |
| F     | 0.00                                | 0.00 | 0.0000 | 0.0000 | 0.0000 | 0.0018 | 0.0000 | COMPARATIVE STEEL |
| G     | 0.00                                | 0.00 | 0.0000 | 0.0000 | 0.0022 | 0.0000 | 0.0000 | PRESENT INVENTION |
| H     | 0.00                                | 0.00 | 0.0000 | 0.0000 | 0.0000 | 0.0000 | 0.0000 | PRESENT INVENTION |
| I     | 0.00                                | 0.00 | 0.0011 | 0.0000 | 0.0000 | 0.0020 | 0.0000 | COMPARATIVE STEEL |
| J     | 0.00                                | 0.00 | 0.0011 | 0.0000 | 0.0000 | 0.0020 | 0.0000 | COMPARATIVE STEEL |
| K     | 0.00                                | 0.00 | 0.0000 | 0.0000 | 0.0000 | 0.0020 | 0.0000 | COMPARATIVE STEEL |
| L     | 0.00                                | 0.00 | 0.0000 | 0.0000 | 0.0000 | 0.0000 | 0.0000 | PRESENT INVENTION |
| M     | 0.00                                | 0.00 | 0.0000 | 0.0000 | 0.0000 | 0.0000 | 0.0000 | PRESENT INVENTION |
| N     | 0.00                                | 0.00 | 0.0010 | 0.0000 | 0.0000 | 0.0000 | 0.0000 | PRESENT INVENTION |
| O     | 0.10                                | 0.00 | 0.0000 | 0.0000 | 0.0000 | 0.0000 | 0.0000 | PRESENT INVENTION |
| P     | 0.00                                | 0.91 | 0.0000 | 0.0000 | 0.0000 | 0.0000 | 0.0000 | PRESENT INVENTION |
| Q     | 0.00                                | 0.00 | 0.0015 | 0.0000 | 0.0000 | 0.0000 | 0.0000 | PRESENT INVENTION |

TABLE 2

| STEEL<br>NUMBER        | COMPONENT | METALLURGICAL FACTORS                                            |                          |                                  |                                     |                                                                           |                                               | MANUFACTURING CONDITIONS                  |                                    |                          |                           |    |  |
|------------------------|-----------|------------------------------------------------------------------|--------------------------|----------------------------------|-------------------------------------|---------------------------------------------------------------------------|-----------------------------------------------|-------------------------------------------|------------------------------------|--------------------------|---------------------------|----|--|
|                        |           | HEATING TEMPERATURE                                              |                          |                                  | ROUGH ROLLING CONDITIONS            |                                                                           |                                               | TIME PERIOD                               |                                    |                          | FINISH ROLLING CONDITIONS |    |  |
|                        |           | Ar <sub>3</sub> TRANSFORMATION<br>POINT<br>TEMPERATURE<br>(° C.) | T <sub>1</sub><br>(° C.) | HEATING<br>TEMPERATURE<br>(° C.) | HEATING<br>TIME<br>PERIOD<br>(° C.) | NUMBER OF TIMES<br>OF REDUCTION<br>AT 100° C. OR HIGHER<br>AT 40% OR MORE | REDUCTION<br>RATIO<br>AT 100° C.<br>OR HIGHER | TO START<br>OF FINISH<br>ROLLING<br>(sec) | TOTAL<br>REDUCTION<br>RATIO<br>(%) | T <sub>f</sub><br>(° C.) | P <sub>1</sub><br>(%)     |    |  |
| PRESENT<br>INVENTION   | 1         | A                                                                | 859                      | 895                              | 1260                                | 45                                                                        | 2                                             | 45/45                                     | 60                                 | 90                       | 990                       | 40 |  |
| PRESENT<br>INVENTION   | 2         | B                                                                | 723                      | 903                              | 1260                                | 45                                                                        | 2                                             | 45/45                                     | 60                                 | 90                       | 990                       | 40 |  |
| COMPARATIVE<br>EXAMPLE | 3         | C                                                                | 720                      | 887                              | 1230                                | 45                                                                        | 3                                             | 40/40/40                                  | 60                                 | 93                       | 980                       | 35 |  |
| COMPARATIVE<br>EXAMPLE | 4         | D                                                                | 798                      | 896                              | 1200                                | 60                                                                        | 3                                             | 40/40/40                                  | 90                                 | 89                       | 990                       | 32 |  |
| EXAMPLE                | 5         | E                                                                | 779                      | 875                              | 1200                                | 60                                                                        | 3                                             | 40/40/40                                  | 90                                 | 89                       | 970                       | 32 |  |
| COMPARATIVE<br>EXAMPLE | 6         | F                                                                | 833                      | 866                              | 1200                                | 60                                                                        | 3                                             | 40/40/40                                  | 90                                 | 89                       | 960                       | 32 |  |
| EXAMPLE                | 7         | G                                                                | 825                      | 851                              | 1200                                | 60                                                                        | 3                                             | 40/40/40                                  | 90                                 | 89                       | 950                       | 32 |  |
| PRESENT<br>INVENTION   | 8         | G                                                                | 825                      | 851                              | 1200                                | 60                                                                        | 0                                             | 25/25/25                                  | 90                                 | 89                       | 950                       | 32 |  |
| COMPARATIVE<br>EXAMPLE | 9         | G                                                                | 825                      | 851                              | 1200                                | 60                                                                        | 3                                             | 40/40/40                                  | 180                                | 89                       | 950                       | 32 |  |
| PRESENT<br>INVENTION   | 10        | G                                                                | 825                      | 851                              | 1200                                | 60                                                                        | 3                                             | 40/40/40                                  | 90                                 | 45                       | 950                       | 32 |  |
| COMPARATIVE<br>EXAMPLE | 11        | G                                                                | 825                      | 851                              | 1200                                | 60                                                                        | 3                                             | 40/40/40                                  | 90                                 | 89                       | 850                       | 32 |  |
| COMPARATIVE<br>EXAMPLE | 12        | G                                                                | 825                      | 851                              | 1200                                | 60                                                                        | 3                                             | 40/40/40                                  | 90                                 | 89                       | 1050                      | 32 |  |
| EXAMPLE                | 13        | G                                                                | 825                      | 851                              | 1200                                | 60                                                                        | 3                                             | 40/40/40                                  | 90                                 | 89                       | 950                       | 29 |  |
| COMPARATIVE<br>EXAMPLE | 14        | G                                                                | 825                      | 851                              | 1200                                | 60                                                                        | 3                                             | 40/40/40                                  | 90                                 | 89                       | 950                       | 32 |  |
| EXAMPLE                | 15        | G                                                                | 825                      | 851                              | 1200                                | 60                                                                        | 3                                             | 40/40/40                                  | 90                                 | 89                       | 950                       | 32 |  |
| COMPARATIVE<br>EXAMPLE | 16        | G                                                                | 825                      | 851                              | 1200                                | 60                                                                        | 3                                             | 40/40/40                                  | 90                                 | 89                       | 950                       | 32 |  |
| COMPARATIVE<br>EXAMPLE | 17        | G                                                                | 825                      | 851                              | 1200                                | 60                                                                        | 3                                             | 40/40/40                                  | 90                                 | 89                       | 950                       | 32 |  |
| EXAMPLE                | 18        | G                                                                | 825                      | 851                              | 1200                                | 60                                                                        | 3                                             | 40/40/40                                  | 90                                 | 89                       | 950                       | 32 |  |
| COMPARATIVE<br>EXAMPLE | 19        | G                                                                | 825                      | 851                              | 1200                                | 60                                                                        | 3                                             | 40/40/40                                  | 90                                 | 89                       | 950                       | 32 |  |
| COMPARATIVE<br>EXAMPLE | 20        | G                                                                | 825                      | 851                              | 1200                                | 60                                                                        | 3                                             | 40/40/40                                  | 90                                 | 89                       | 950                       | 32 |  |

TABLE 2-continued

| MANUFACTURING CONDITIONS           |                                      |                           |                                               |                     |     |                                 |     |     |                                                 |    |     |
|------------------------------------|--------------------------------------|---------------------------|-----------------------------------------------|---------------------|-----|---------------------------------|-----|-----|-------------------------------------------------|----|-----|
| FINISH ROLLING                     |                                      |                           |                                               |                     |     | COOLING CONDITIONS              |     |     |                                                 |    |     |
| CONDITIONS                         |                                      |                           | TIME PERIOD TO START OF PRIMARY COOLING (sec) |                     |     | PRIMARY COOLING RATE (° C./sec) |     |     | TIME PERIOD TO START OF SECONDARY COOLING (sec) |    |     |
| MAXIMUM WORKING TEMPERATURE (° C.) | HEAT GENERATION t <sub>1</sub> (sec) | t <sub>1</sub> -2.5 (sec) | t <sub>1</sub>                                | t <sub>1</sub> -2.5 | 1.0 | 2.5                             | 135 | 90  | 1.5                                             | 30 | 660 |
| PRESENT INVENTION                  | 15                                   | 0.40                      | 1.00                                          | 1.0                 | 2.0 | 60                              | 90  |     | 2.5                                             | 30 | 660 |
| PRESENT INVENTION                  | 12                                   | 0.51                      | 1.28                                          | 1.0                 | 2.0 | 60                              | 90  |     | 2.5                                             | 30 | 660 |
| COMPARATIVE EXAMPLE                | 15                                   | 0.62                      | 1.55                                          | 0.8                 | 1.3 | 65                              | 110 | 1.0 | 40                                              | 40 | 680 |
| COMPARATIVE EXAMPLE                | 12                                   | 0.73                      | 1.83                                          | 0.9                 | 1.2 | 60                              | 70  | 1.6 | 25                                              | 25 | 680 |

TABLE 2-continued

|                     |    |      |      |            |            |          |            |             |    |            |   |     |
|---------------------|----|------|------|------------|------------|----------|------------|-------------|----|------------|---|-----|
| COMPARATIVE EXAMPLE | 12 | 0.71 | 1.79 | 0.9        | 1.3        | 60       | 70         | 1.6         | 25 | 670        | 2 | 470 |
| COMPARATIVE EXAMPLE | 12 | 0.72 | 1.81 | 0.9        | 1.2        | 60       | 70         | 1.6         | 25 | 690        | 2 | 470 |
| PRESENT INVENTION   | 12 | 0.65 | 1.63 | 0.9        | 1.4        | 45       | 70         | 1.6         | 25 | 700        | 4 | 500 |
| COMPARATIVE EXAMPLE | 12 | 0.65 | 1.63 | 0.9        | 1.4        | 60       | 70         | 1.6         | 25 | 700        | 4 | 500 |
| PRESENT INVENTION   | 12 | 0.65 | 1.63 | 0.9        | 1.4        | 60       | 70         | 1.6         | 25 | 700        | 4 | 500 |
| COMPARATIVE EXAMPLE | 12 | 0.65 | 1.63 | 0.9        | 1.4        | 60       | 70         | 1.6         | 25 | 700        | 4 | 500 |
| COMPARATIVE EXAMPLE | 12 | 0.21 | 0.53 | 0.9        | 4.2        | 60       | 70         | 1.6         | 25 | 700        | 4 | 500 |
| COMPARATIVE EXAMPLE | 12 | —    | —    | 0.9        | —          | 60       | 70         | 1.6         | 25 | 700        | 4 | 500 |
| COMPARATIVE EXAMPLE | 25 | 0.65 | 1.63 | 0.9        | 1.4        | 60       | 70         | 1.6         | 25 | 700        | 4 | 500 |
| COMPARATIVE EXAMPLE | 12 | 0.65 | 1.63 | <u>2.0</u> | <u>3.1</u> | 60       | 70         | 1.6         | 25 | 700        | 4 | 500 |
| COMPARATIVE EXAMPLE | 12 | 0.65 | 1.63 | 0.9        | 1.4        | <u>5</u> | 70         | 1.6         | 25 | 700        | 4 | 500 |
| COMPARATIVE EXAMPLE | 12 | 0.65 | 1.63 | 0.9        | 1.4        | 60       | <u>20</u>  | 1.6         | 25 | 700        | 4 | 500 |
| COMPARATIVE EXAMPLE | 12 | 0.65 | 1.63 | 0.9        | 1.4        | 60       | <u>200</u> | 1.6         | 25 | 700        | 4 | 500 |
| COMPARATIVE EXAMPLE | 12 | 0.65 | 1.63 | 0.9        | 1.4        | 60       | 70         | <u>10.0</u> | 25 | 700        | 4 | 500 |
| COMPARATIVE EXAMPLE | 12 | 0.65 | 1.63 | 0.9        | 1.4        | 60       | 70         | 1.6         | 25 | <u>840</u> | 4 | 500 |
| COMPARATIVE EXAMPLE | 12 | 0.65 | 1.63 | 0.9        | 1.4        | 60       | 70         | 1.6         | 25 | <u>580</u> | 4 | 500 |
| COMPARATIVE EXAMPLE | 12 | 0.65 | 1.63 | 0.9        | 1.4        | 60       | 70         | 1.6         | 25 | —          | — | 500 |
| COMPARATIVE EXAMPLE | 12 | 0.65 | 1.63 | 0.9        | 1.4        | 60       | 70         | 1.6         | 25 | 700        | 2 | 530 |
| COMPARATIVE EXAMPLE | 12 | 0.65 | 1.63 | 0.9        | 1.4        | 60       | 70         | 1.6         | 25 | 670        | 2 | 530 |
| COMPARATIVE EXAMPLE | 12 | 0.89 | 2.22 | 0.9        | 1.0        | 60       | 70         | 1.0         | 20 | 670        | 2 | 530 |
| COMPARATIVE EXAMPLE | 12 | 0.88 | 2.19 | 0.9        | 1.0        | 60       | 70         | 1.0         | 20 | 670        | 2 | 530 |
| COMPARATIVE EXAMPLE | 12 | 0.82 | 2.05 | 0.9        | 1.1        | 60       | 70         | 1.0         | 20 | 670        | 2 | 530 |

TABLE 2-continued

|           |    |      |      |     |     |    |    |     |    |     |    |     |
|-----------|----|------|------|-----|-----|----|----|-----|----|-----|----|-----|
| PRESENT   | 12 | 0.61 | 1.52 | 0.9 | 1.5 | 60 | 70 | 1.0 | 20 | 670 | 10 | 470 |
| INVENTION | 12 | 0.73 | 1.83 | 0.9 | 1.2 | 60 | 70 | 1.0 | 20 | 670 | 10 | 470 |
| PRESENT   | 12 | 2.00 | 5.00 | 0.9 | 0.5 | 60 | 70 | 1.0 | 20 | 670 | 10 | 470 |
| INVENTION | 12 | 0.99 | 2.47 | 0.9 | 0.9 | 60 | 70 | 1.0 | 20 | 670 | 10 | 470 |
| PRESENT   | 12 | 1.08 | 2.71 | 0.9 | 0.8 | 60 | 70 | 1.0 | 20 | 670 | 10 | 470 |
| INVENTION | 12 | 0.81 | 2.03 | 0.7 | 0.9 | 60 | 70 | 1.0 | 20 | 670 | 10 | 470 |

In Table 2, "COMPONENT" means the symbol of steel shown in Table 1. "Ar3 TRANSFORMATION POINT TEMPERATURE" is the temperature calculated by Expressions (6), (7), and (8) above. "T1" indicates the temperature calculated by Expression (1) above. "t1" indicates the temperature calculated by Expression (2) above.

"HEATING TEMPERATURE" is the heating temperature in the heating process. "HOLDING TIME PERIOD" is the holding time period at a predetermined heating temperature in the heating process.

from the completion of the secondary cooling to the coiling. "AIR COOLING HOLDING TIME PERIOD" is the holding time period when the holding (air cooling) is performed. "COILING TEMPERATURE" is the temperature at which the steel sheet is coiled by a coiler in the coiling process.

Further, with regard to the present invention example of Steel number 7 and the comparative examples of Steel numbers 13 and 10, the relationship between, of the finish rolling, the reduction ratio of each of rolling stands F1 to F7 and the temperature region is shown in Table 4.

TABLE 3

|                     | F1   | F2   | F3   | F4   | F5   | F6   | F7   | TOTAL REDUCTION RATIO AT T1 + 30° C. OR HIGHER |
|---------------------|------|------|------|------|------|------|------|------------------------------------------------|
| PRESENT INVENTION   | 38.9 | 37.8 | 37.4 | 34.7 | 31.9 | 0.0  | 0.0  | 89                                             |
| COMPARATIVE EXAMPLE | 29.0 | 28.8 | 28.8 | 27.5 | 26.6 | 25.9 | 25.6 | 89                                             |
| COMPARATIVE EXAMPLE | 0.0  | 19.1 | 32.4 | 32.3 | 32.1 | 34.2 | 36.0 | 45                                             |

"NUMBER OF TIMES OF REDUCTION AT 1000° C. OR HIGHER AT 40% OR MORE" is the number of times of reduction at a reduction ratio of 40% or more in the temperature range of not lower than 1000° C. nor higher than 1200° C. in the rough rolling. "REDUCTION RATIO AT 1000° C. OR HIGHER" is each reduction ratio (reduction pass schedule) in the temperature range of not lower than 1000° C. nor higher than 1200° C. in the rough rolling. It is indicated that in a present invention example (Steel number 1), for example, the reduction at a reduction ratio of 45% was performed two times. Further, it is indicated that in a comparative example (Steel number 3), for example, the reduction at a reduction ratio of 40% was performed three times. "TIME PERIOD TO START OF FINISH ROLLING" is the time period from the completion of the rough rolling process to the start of the finish rolling process. "TOTAL REDUCTION RATIO" is the total reduction ratio in the finish rolling process.

"Tf" indicates the temperature after the final reduction at 30% or more in the finish rolling. "P1" indicates the reduction ratio of the final reduction at 30% or more in the finish rolling. However, in the comparative example (Steel number 13), the largest value among the reduction ratios of the respective rolling stands 6 in the finish rolling was 29%. In the comparative example (Steel number 13), the temperature after the reduction at this reduction ratio of 29% was set to "Tf." "MAXIMUM WORKING HEAT GENERATION" is the maximum temperature increased by the heat generation by working between respective finishing passes (between the respective rolling stands 6).

"TIME PERIOD TO START OF PRIMARY COOLING" is the time period from after the completion of the final reduction at 30% or more in the finish rolling to the start of the primary cooling. "PRIMARY COOLING RATE" is the average cooling rate to which the cooling corresponding to the amount of the primary cooling temperature change is completed. "PRIMARY COOLING TEMPERATURE CHANGE" is the difference between, of the primary cooling, the start temperature and the finishing temperature.

"TIME PERIOD TO START OF SECONDARY COOLING" is the time period from the completion of the primary cooling to the start of the secondary cooling. "SECONDARY COOLING RATE" is the average cooling rate from the start of the secondary cooling to the coiling, from which the holding time period (air cooling time period) is removed. "AIR COOLING TEMPERATURE REGION" is the temperature region where the holding (air cooling) is performed

20 In the present invention example of Steel number 7, the steel sheet was in the temperature region of not lower than T1+30° C. nor higher than T1+200° C. at the rolling stands F1 to F5, and was in the temperature region of lower than T1+30° C. at and after the rolling stand F6. In the present invention example of Steel number 7, at the rolling stands F1 to F5, the reduction at a reduction ratio of 30% or more was performed five times in the temperature region of not lower than T1+30° C. nor higher than T1+200° C., and after the 25 rolling stand F6, no reduction was performed practically in the temperature region of lower than T1+30° C. The steel sheet was just passed through the rolling stands F6 and F7. As was shown also in Table 2, in the present invention example of Steel number 7, the total reduction ratio in the temperature region of not lower than T1+30° C. nor higher than T1+200° C. is 89%.

Incidentally, the reduction ratio at each of the rolling stands F1 to F7 is obtained by the change in sheet thickness between the entry side and the exist side of each of the 30 rolling stands F1 to F7. In contrast to this, the total reduction ratio in the temperature region of not lower than T1+30° C. nor higher than T1+200° C. is obtained by the change in sheet thickness before and after all the rolling passes performed in the temperature region in the finish rolling. As 35 shown in the present invention example of Steel number 7, for example, the total reduction ratio in the temperature region is obtained by the change in sheet thickness before and after all the rolling passes performed at the rolling stands F1 to F5. That is, it is obtained by the change between the 40 sheet thickness on the entry side of the rolling stand F1 and the sheet thickness on the exist side of the rolling stand F5.

On the other hand, in the comparative example of Steel number 13, the steel sheet was in the temperature region of not lower than T1+30° C. nor higher than T1+200° C. at all 45 the rolling stands F1 to F7 in the finish rolling. As was shown also in Table 2, in the comparative example of steel number 13, the total reduction ratio in the temperature region of not lower than T1+30° C. nor higher than T1+200° C. is 89%. However, in the comparative example of Steel 50 number 13, at each of the rolling stands F1 to F7, the reduction at a reduction ratio of 30% or more is not performed.

Further, in the comparative example of Steel number 10, the steel sheet was in the temperature region of not lower than T1+30° C. nor higher than T1+200° C. at the rolling 55 stands F1 to F3, and the steel sheet was in the temperature region of lower than T1+30° C. at and after the rolling stand

F4. In the comparative example of Steel number 10, at the rolling stands F1 to F3, the reduction at a reduction ratio of 30% or more was performed three times in the temperature region of not lower than T1+30° C. nor higher than T1+200° C., and further also in the temperature region of lower than T1+30° C. at and after the rolling stand F4, the reduction at a reduction ratio of 30% or more was performed four times.

As was shown also in Table 2, in the comparative example of steel number 10, the total reduction ratio in the temperature region of not lower than T1+30° C. nor higher than T1+200° C. is 45%.

The evaluation methods of the obtained hot-rolled steel sheet are the same as the previously described methods. Evaluation results are shown in Table 3.

TABLE 4

| STEEL NUMBER        | STRUCTURAL FRACTION | GRAIN DIAMETER (μm) | MICROSTRUCTURE  |                                                                               |                                                |
|---------------------|---------------------|---------------------|-----------------|-------------------------------------------------------------------------------|------------------------------------------------|
|                     |                     |                     | AVERAGE CRYSTAL | AVERAGE VALUE OF POLE DENSITIES OF {100}<011> TO {223}<110> ORIENTATION GROUP | POLE DENSITY OF {332}<113> CRYSTAL ORIENTATION |
| PRESENT INVENTION   | 1                   | Zw + 8% F           | 7.5             | 1.7                                                                           | 2.5                                            |
| PRESENT INVENTION   | 2                   | Zw + 6% F           | 8.0             | 1.7                                                                           | 2.5                                            |
| COMPARATIVE EXAMPLE | 3                   | Zw                  | 8.0             | 1.8                                                                           | 2.6                                            |
| COMPARATIVE EXAMPLE | 4                   | Zw                  | 7.0             | 1.7                                                                           | 2.5                                            |
| COMPARATIVE EXAMPLE | 5                   | Zw                  | 9.0             | 2.0                                                                           | 2.9                                            |
| COMPARATIVE EXAMPLE | 6                   | Zw +36% F           | 8.0             | 2.0                                                                           | 2.9                                            |
| PRESENT INVENTION   | 7                   | Zw + 32% F          | 9.5             | 2.0                                                                           | 2.9                                            |
| COMPARATIVE EXAMPLE | 8                   | Zw + 28% F          | 10.5            | 1.7                                                                           | 2.5                                            |
| PRESENT INVENTION   | 9                   | Zw + 30% F          | 10.0            | 3.1                                                                           | 4.2                                            |
| COMPARATIVE EXAMPLE | 10                  | Zw + 34% F          | 7.0             | 4.2                                                                           | 5.0                                            |
| COMPARATIVE EXAMPLE | 11                  | Zw + 33% F          | 4.5             | 5.1                                                                           | 5.5                                            |
| COMPARATIVE EXAMPLE | 12                  | Zw + 26% F          | 11.0            | 1.7                                                                           | 2.5                                            |
| COMPARATIVE EXAMPLE | 13                  | Zw + 31% F          | 6.5             | 5.3                                                                           | 5.6                                            |
| COMPARATIVE EXAMPLE | 14                  | Zw + 35% F          | 10.5            | 1.7                                                                           | 2.5                                            |
| COMPARATIVE EXAMPLE | 15                  | Zw + 34% F          | 12.0            | 1.7                                                                           | 2.5                                            |
| COMPARATIVE EXAMPLE | 16                  | Zw + 33% F          | 11.5            | 1.8                                                                           | 2.6                                            |
| COMPARATIVE EXAMPLE | 17                  | Zw + 34% F          | 10.5            | 1.8                                                                           | 2.6                                            |
| COMPARATIVE EXAMPLE | 18                  | Zw + 33% F          | 6.5             | 5.4                                                                           | 5.7                                            |
| COMPARATIVE EXAMPLE | 19                  | P +44% F            | 8.5             | 1.9                                                                           | 2.8                                            |
| COMPARATIVE EXAMPLE | 20                  | P +38% F            | 8.0             | 2.0                                                                           | 2.9                                            |
| COMPARATIVE EXAMPLE | 21                  | P +45% F            | 8.5             | 2.0                                                                           | 2.9                                            |
| COMPARATIVE EXAMPLE | 22                  | Zw                  | 8.0             | 2.0                                                                           | 2.9                                            |
| COMPARATIVE EXAMPLE | 23                  | Zw                  | 8.5             | 2.0                                                                           | 2.9                                            |
| COMPARATIVE EXAMPLE | 24                  | P +47% F            | 8.5             | 2.0                                                                           | 2.9                                            |
| COMPARATIVE EXAMPLE | 25                  | 56% F +M            | 8.5             | 2.0                                                                           | 2.9                                            |
| COMPARATIVE EXAMPLE | 26                  | P +37% F            | 8.5             | 2.0                                                                           | 2.9                                            |
| PRESENT INVENTION   | 27                  | Zw + 15% F          | 8.0             | 1.8                                                                           | 2.6                                            |
| COMPARATIVE EXAMPLE | 28                  | 67% F +Zw           | 8.5             | 2.0                                                                           | 2.9                                            |
| COMPARATIVE EXAMPLE | 29                  | F                   | 11.0            | 2.0                                                                           | 2.9                                            |
| COMPARATIVE EXAMPLE | 30                  | Zw                  | 9.5             | 2.6                                                                           | 3.7                                            |
| PRESENT INVENTION   | 31                  | Zw + 8% F           | 6.5             | 2.0                                                                           | 2.9                                            |
| PRESENT INVENTION   | 32                  | Zw + 11% F          | 7.5             | 1.9                                                                           | 2.8                                            |
| PRESENT INVENTION   | 33                  | Zw + 9% F           | 6.0             | 3.9                                                                           | 2.8                                            |
| PRESENT INVENTION   | 34                  | Zw + 17% F          | 4.0             | 3.6                                                                           | 2.6                                            |
| PRESENT INVENTION   | 35                  | Zw + 14% F          | 6.5             | 3.7                                                                           | 2.6                                            |
| PRESENT INVENTION   | 36                  | Zw + 14% F          | 6.5             | 3.3                                                                           | 2.8                                            |

## MECHANICAL PROPERTIES

|                     | TENSILE TEST |             |           | ISOTROPY<br>1/ Δr | λ<br>(%) | HOLE<br>EXPANSION | BENDABILITY | MINIMUM<br>BEND RADIUS | TOUGHNESS<br>vTrs(° C.) |
|---------------------|--------------|-------------|-----------|-------------------|----------|-------------------|-------------|------------------------|-------------------------|
|                     | YP<br>(MPa)  | TS<br>(MPa) | EI<br>(%) |                   |          |                   |             |                        |                         |
| PRESENT INVENTION   | 906          | 998         | 15        | 12.5              | 71       | 0.6               |             | -58                    |                         |
| PRESENT INVENTION   | 857          | 1015        | 14        | 12.5              | 75       | 0.5               |             | -48                    |                         |
| COMPARATIVE EXAMPLE | 677          | 744         | 11        | 9.2               | 71       | 0.6               |             | -48                    |                         |
| COMPARATIVE EXAMPLE | 700          | 761         | 10        | 12.5              | 70       | 0.8               |             | -68                    |                         |
| COMPARATIVE EXAMPLE | 716          | 770         | 9         | 6.5               | 70       | 0.8               |             | -31                    |                         |
| COMPARATIVE EXAMPLE | 412          | 588         | 28        | 6.5               | 68       | 1.1               |             | -48                    |                         |
| PRESENT INVENTION   | 475          | 577         | 30        | 6.5               | 131      | 0.2               |             | -25                    |                         |
| COMPARATIVE EXAMPLE | 484          | 580         | 28        | 12.5              | 125      | 0.1               |             | -11                    |                         |
| PRESENT INVENTION   | 490          | 588         | 27        | 3.8               | 123      | 0.1               |             | -20                    |                         |
| COMPARATIVE EXAMPLE | 482          | 581         | 28        | 3.2               | 88       | 0.2               |             | -68                    |                         |
| COMPARATIVE EXAMPLE | 475          | 575         | 28        | 3.1               | 87       | 0.2               |             | -125                   |                         |
| COMPARATIVE EXAMPLE | 458          | 560         | 29        | 12.5              | 132      | 0.1               |             | -5                     |                         |
| COMPARATIVE EXAMPLE | 477          | 577         | 28        | 3.0               | 85       | 0.1               |             | -80                    |                         |
| COMPARATIVE EXAMPLE | 480          | 571         | 28        | 12.5              | 136      | 0.2               |             | -17                    |                         |
| COMPARATIVE EXAMPLE | 478          | 585         | 26        | 12.5              | 135      | 0.2               |             | 6                      |                         |
| COMPARATIVE EXAMPLE | 481          | 579         | 27        | 9.2               | 130      | 0.1               |             | 0                      |                         |
| COMPARATIVE EXAMPLE | 471          | 577         | 27        | 9.2               | 133      | 0.2               |             | -17                    |                         |
| COMPARATIVE EXAMPLE | 468          | 566         | 28        | 3.0               | 89       | 0.2               |             | -80                    |                         |

TABLE 4-continued

|                     |     |             |           |     |           |            |           |
|---------------------|-----|-------------|-----------|-----|-----------|------------|-----------|
| COMPARATIVE EXAMPLE | 420 | <u>521</u>  | 24        | 7.5 | 67        | <u>1.4</u> | -40       |
| COMPARATIVE EXAMPLE | 418 | <u>520</u>  | 25        | 6.5 | 65        | <u>1.7</u> | -48       |
| COMPARATIVE EXAMPLE | 409 | <u>510</u>  | 26        | 6.5 | 66        | <u>1.8</u> | -40       |
| COMPARATIVE EXAMPLE | 581 | 644         | <u>15</u> | 6.5 | 76        | 0.9        | -48       |
| COMPARATIVE EXAMPLE | 601 | 650         | <u>14</u> | 6.5 | 75        | 0.8        | -40       |
| COMPARATIVE EXAMPLE | 390 | <u>495</u>  | 27        | 6.5 | 69        | <u>1.6</u> | -40       |
| COMPARATIVE EXAMPLE | 370 | 622         | 28        | 6.5 | <u>41</u> | <u>2.1</u> | -40       |
| COMPARATIVE EXAMPLE | 400 | <u>503</u>  | 26        | 6.5 | 69        | <u>1.8</u> | -40       |
| PRESENT INVENTION   | 548 | 655         | 26        | 9.2 | 141       | 0.1        | -48       |
| COMPARATIVE EXAMPLE | 396 | <u>522</u>  | 30        | 6.5 | 122       | <u>1.1</u> | -40       |
| COMPARATIVE EXAMPLE | 355 | <u>462</u>  | 35        | 6.5 | 140       | 0.1        | <u>-5</u> |
| COMPARATIVE EXAMPLE | 986 | <u>1126</u> | <u>5</u>  | 4.3 | <u>22</u> | 0.8        | -24       |
| PRESENT INVENTION   | 588 | 711         | 24        | 6.5 | 105       | 0.1        | -80       |
| PRESENT INVENTION   | 570 | 702         | 25        | 7.5 | 97        | 0.08       | -58       |
| PRESENT INVENTION   | 592 | 720         | 24        | 4.8 | 101       | 0.1        | -93       |
| PRESENT INVENTION   | 585 | 700         | 25        | 4.6 | 96        | 0.07       | -127      |
| PRESENT INVENTION   | 578 | 695         | 25        | 4.7 | 93        | 0.1        | -80       |
| PRESENT INVENTION   | 603 | 732         | 23        | 4.3 | 91        | 0.1        | -80       |

"STRUCTURAL FRACTION" is the area fraction of each structure measured by a point counting method from an optical microscope structure. "AVERAGE CRYSTAL GRAIN DIAMETER" is the average crystal grain diameter measured by the EBSP-OIM™.

"AVERAGE VALUE OF X-RAY RANDOM INTENSITIES OF {100}<011> TO {223}<110> ORIENTATION GROUP" is the pole density of the {100}<011> to {223}<110> orientation group parallel to the rolled plane. "POLE DENSITY OF {332}<113> CRYSTAL ORIENTATION" is the pole density of the {332}<113> crystal orientation parallel to the rolled plane.

"TENSILE TEST" indicates the result obtained after a tensile test being performed on a C-direction JIS No. 5 test piece. "YP" indicates the yield point, "TS" indicates the tensile strength, and "EL" indicates the elongation.

"ISOTROPY" indicates the inverse number of  $|\Delta r|$  as an index. "HOLE EXPANSION  $\lambda$ " indicates the result obtained by the hole expanding test method described in JIS T 1001-1996. "BENDABILITY (MINIMUM BEND RADIUS)" indicates the result obtained by performing a test using a No. 1 test piece ( $t \times 40$  mm  $W \times 80$  mm  $L$ ), at a pressing jig speed of 0.1 m/second, in accordance with the pressing bend method (roller bend method) described in JIS Z 2248.  $YP \geq 320$  MPa,  $TS \geq 540$  MPa,  $EL \geq 18\%$ ,  $\lambda \geq 70\%$ , and the minimum bend radius  $\leq 1$  mm were accepted.

Incidentally, a length  $L$  between supporting points is  $L = 2r + 3t$ , where the sheet thickness is set to  $t$  (mm) and the inside radius of a tip of the pressing jig is set to  $r$  (mm).

In this method, a bending angle was set up to 170°, and thereafter an interposed object having a thickness twice as large as the radius of the pressing jig was used, the test piece was pressed against the interposed object to be wound therearound, and with a bending angle of 180°, cracking in the outside of a bent portion was observed visually.

"MINIMUM BEND RADIUS" is one that the test is performed by decreasing the inside radius  $r$  (mm) until cracking occurs and the minimum inside radius  $r$  (mm) that does not cause cracking is divided by the sheet thickness  $t$  (mm) to be made dimensionless by  $r/t$ . "MINIMUM BEND RADIUS" becomes the smallest in the case of close-contact bending that is performed without the interposed object, and in the case, "MINIMUM BEND RADIUS" is zero. Incidentally, a bending direction was set at 45° from the rolling direction. "TOUGHNESS" is indicated by the transition temperature obtained by a subsize V-notch Charpy test.

The invention examples correspond to the nine examples of Steel numbers 1, 2, 7, 27, and 31 to 35. In these invention

examples of Steel numbers, the high-strength steel sheet in which the texture of the steel sheet having a required chemical composition is obtained, the average value of the pole densities of the {100}<011> to {223}<110> orientation group of the sheet plane at a sheet thickness of  $\frac{5}{8}$  to  $\frac{3}{8}$  from the surface of the steel sheet is at least 4.0 or less, the pole density of the {332}<113> crystal orientation is 4.8 or less, and the average crystal grain diameter at the sheet thickness center is 9  $\mu\text{m}$  or less, the microstructure is composed of pro-eutectoid ferrite in a structural fraction of 35% or less at the sheet thickness center and the low-temperature transformation generating phase, and the tensile strength is 540 MPa class or more is obtained.

The comparative examples of the steel sheet other than the above-described examples each fall outside the range of the present invention due to the following reasons.

With regard to Steel numbers 3 to 5, the C content is outside the range of the present invention, and thus the microstructure is outside the range of the present invention and the elongation is poor. With regard to Steel number 6, the C content is outside the range of the present invention, and thus the microstructure is outside the range of the present invention and the bendability is poor.

With regard to Steel number 8, the number of times of the reduction at 1000°C. or higher at 35% or more in the rough rolling is outside the range of the present invention, and thus the average crystal grain diameter is outside the range of the present invention and the toughness is poor. With regard to Steel number 9, the time period to the start of the finish rolling is long, the average crystal grain diameter is outside the range of the present invention, and the toughness is poor.

With regard to Steel number 10, the average value of the pole densities of the {100}<011> to {223}<110> orientation group and the pole density of the {332}<113> crystal orientation are both outside the range of the present invention and the isotropy is low.

With regard to Steel number 11, the value of  $T_f$  is outside the range of the present invention, and thus the average value of the pole densities of the {100}<011> to {223}<110> orientation group and the pole density of the {332}<113> crystal orientation are both outside the range of the present invention and the isotropy is low.

With regard to Steel number 12, the value of  $T_f$  is outside the range of the present invention, and thus the average crystal grain diameter is outside the range of the present invention and the toughness is poor. With regard to Steel number 13, the value of  $P_1$  is outside the range of the present invention and at each of the rolling stands  $F_1$  to  $F_7$  in the

41

finish rolling, the reduction at a reduction ratio of 30% or more was not performed, and thus the average value of the pole densities of the  $\{100\}<011>$  to  $\{223\}<110>$  orientation group and the pole density of the  $\{332\}<113>$  crystal orientation are both outside the range of the present invention and the isotropy is low.

With regard to Steel number 14, the maximum working heat generation temperature is outside the range of the present invention, and thus the average crystal grain diameter is outside the range of the present invention and the toughness is poor. With regard to Steel number 15, the time period to the primary cooling is outside the range of the present invention, and thus the average crystal grain diameter is outside the range of the present invention and the toughness is poor. With regard to Steel number 16, the primary cooling rate is outside the range of the present invention, and thus the average crystal grain diameter is outside the range of the present invention and the toughness is poor.

With regard to Steel number 17, the primary cooling temperature change is outside the range of the present invention, and thus average crystal grain diameter is outside the range of the present invention and the toughness is poor. With regard to Steel number 18, the primary cooling temperature change is outside the range of the present invention, and thus the average value of the pole densities of the  $\{100\}<011>$  to  $\{223\}<110>$  orientation group and the pole density of the  $\{332\}<113>$  crystal orientation are both outside the range of the present invention and the isotropy is low.

With regard to Steel number 19, the time period to the secondary cooling is outside the range of the present invention, and thus the microstructure is outside the range of the present invention, the strength is low, and the bendability is poor. With regard to Steel number 20, the secondary cooling rate is outside the range of the present invention, and thus the microstructure is outside the range of the present invention, the strength is low, and the bendability is poor.

With regard to Steel number 21, the air cooling temperature region is outside the range of the present invention, and thus the microstructure is outside the range of the present invention, the strength is low, and the bendability is poor.

With regard to Steel number 22, the air cooling temperature region is outside the range of the manufacturing method of the hot-rolled steel sheet of the present invention, and thus the microstructure is outside the range of the present invention and the elongation is poor. With regard to Steel number 23, the air cooling temperature holding time period is outside the range of the present invention, and thus the microstructure is outside the range of the present invention and the elongation is poor. With regard to Steel number 24, the air cooling temperature holding time period is outside the range of the present invention, and thus the microstructure is outside the range of the present invention, the strength is low, and the bendability is poor.

With regard to Steel number 25, the cooling temperature is outside the range of the present invention, and thus the microstructure is outside the range of the present invention and the bendability is poor. With regard to Steel number 26, the cooling temperature is outside the range of the present invention, and thus the microstructure is outside the range of the present invention, the strength is low, and the bendability is poor.

With regard to Steel number 28, the C content is outside the range of the present invention, and thus the microstructure is outside the range of the present invention, the strength is low, and the bendability is poor. With regard to Steel

42

number 29, the C content is outside the range of the present invention, and thus the microstructure is outside the range of the present invention, the strength is low, and the bendability is poor. With regard to Steel number 30, the C content is outside the range of the present invention, and thus the microstructure is outside the range of the present invention and the elongation is poor.

## INDUSTRIAL APPLICABILITY

As has been described previously, according to the present invention, it is possible to easily provide a steel sheet applicable to a member required to have workability, hole expandability, bendability, strict sheet thickness uniformity and circularity after working, and low-temperature toughness (an inner sheet member, a structure member, an under-body member, an automobile member such as a transmission, and members for shipbuilding, construction, bridges, offshore structures, pressure vessels, line pipes, and machine parts, and so on). Further, according to the present invention, it is possible to manufacture a high-strength steel sheet having excellent low-temperature toughness and 540 MPa class or more inexpensively and stably. Thus, the present invention is the invention having high industrial value.

## EXPLANATION OF CODES

1 continuous hot rolling line

2 roughing mill

3 finishing mill

4 hot-rolled steel sheet

5 run-out-table

6 rolling stand

10 inter-stand cooling nozzle

11 cooling nozzle 11

What is claimed is:

1. A bainite-containing high-strength hot-rolled steel sheet, comprising: in mass %,  
C: greater than 0.07 to 0.2%;  
Si: 0.001 to 2.5%;  
Mn: 0.01 to 4%;  
P: 0.15% or less (not including 0%);  
S: 0.03% or less (not including 0%);  
N: 0.01% or less (not including 0%);  
Al: 0.001 to 2%; and

a balance being composed of Fe and inevitable impurities, wherein an average value of pole densities of the  $\{100\}<011>$  to  $\{223\}<110>$  orientation group represented by respective crystal orientations of  $\{100\}<011>$ ,  $\{116\}<110>$ ,  $\{114\}<110>$ ,  $\{113\}<110>$ ,  $\{112\}<110>$ ,  $\{335\}<110>$ , and  $\{223\}<110>$  at a sheet thickness center portion being a range of  $\frac{5}{8}$  to  $\frac{3}{8}$  in sheet thickness from the surface of the steel sheet is 4.0 or less, and a pole density of the  $\{332\}<113>$  crystal orientation is 4.8 or less, an average crystal grain diameter is 10  $\mu\text{m}$  or less and a Charpy fracture appearance transition temperature  $\text{vTrs}$  is  $-20^\circ\text{C}$ . or lower, and a microstructure is composed of 35% or less in a structural fraction of pro-eutectoid ferrite and a balance of a low-temperature transformation generating phase.

2. The bainite-containing high-strength hot-rolled steel sheet according to claim 1, further comprising:  
one or two or more of in mass %,  
Ti: 0.015 to 0.18%,  
Nb: 0.005 to 0.06%,  
Cu: 0.02 to 1.2%,

Ni: 0.01 to 0.6%,

Mo: 0.01 to 1%,

V: 0.01 to 0.2%, and Cr: 0.01 to 2%.

3. The bainite-containing high-strength hot-rolled steel sheet according to claim 1, further comprising:

5

one or two or more of in mass %,

Mg: 0.0005 to 0.01%,

Ca: 0.0005 to 0.01%, and REM: 0.0005 to 0.1%.

4. The bainite-containing high-strength hot-rolled steel sheet according to claim 1, further comprising: in mass %, 10

B: 0.0002 to 0.002%.

\* \* \* \* \*